



US006316173B1

(12) **United States Patent**  
Irving et al.

(10) **Patent No.:** **US 6,316,173 B1**  
(45) **Date of Patent:** **Nov. 13, 2001**

(54) **SHEET COMPRISING AN ION EXCHANGES REDUCING AGENT AND METHODS OF PROCESSING PHOTOGRAPHIC ELEMENTS IN THE PRESENCE OF SAID SHEET**

(75) Inventors: **Lyn M. Irving; Mark E. Irving; John M. Noonan**, all of Rochester, NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/593,087**

(22) Filed: **Jun. 13, 2000**

(51) **Int. Cl.<sup>7</sup>** ..... **G03C 5/26; G03C 7/30**

(52) **U.S. Cl.** ..... **430/404**

(58) **Field of Search** ..... 430/404

(56) **References Cited**

U.S. PATENT DOCUMENTS

3,342,599 9/1967 Reeves ..... 430/311

|           |           |                  |       |         |
|-----------|-----------|------------------|-------|---------|
| 4,060,418 | 11/1977   | Waxman et al.    | ..... | 430/212 |
| 4,157,915 | 6/1979    | Hamaoka et al.   | ..... | 430/505 |
| 4,438,195 | 3/1984    | Kunitz et al.    | ..... | 430/566 |
| 4,490,461 | * 12/1984 | Webb et al.      | ..... | 430/566 |
| 5,019,492 | 5/1991    | Buchanan et al.  | ..... | 430/543 |
| 5,240,821 | * 8/1993  | Texter et al.    | ..... | 430/405 |
| 5,695,916 | * 12/1997 | Fyson            | ..... | 430/403 |
| 5,763,148 | * 6/1998  | Willem et al.    | ..... | 430/405 |
| 5,972,555 | * 10/1999 | Fernandez-Puente | ..... | 430/138 |
| 5,976,773 | * 11/1999 | Fernandez-Puente | ..... | 430/404 |
| 6,136,495 | * 10/2000 | Sakata           | ..... | 430/203 |

\* cited by examiner

Primary Examiner—Hoa Van Le

(74) Attorney, Agent, or Firm—Edith A. Rice

(57) **ABSTRACT**

This invention comprises a sheet comprising at least one photographically useful reducing agent ionically bound to an ion exchange matrix. In preferred embodiments of the invention, the sheet further comprises a binder and/or support and the ion exchange matrix comprises particles having an average particle size of less than about 10 micrometers ( $\mu\text{m}$ ). This invention further comprises methods or processing photographic elements using said sheet.

**33 Claims, 2 Drawing Sheets**

FIG. 1



FIG. 2



**SHEET COMPRISING AN ION EXCHANGES  
REDUCING AGENT AND METHODS OF  
PROCESSING PHOTOGRAPHIC ELEMENTS  
IN THE PRESENCE OF SAID SHEET**

**FIELD OF THE INVENTION**

This invention pertains to a sheet comprising a reducing agent ionically bound to an ion exchange matrix and to methods of processing photographic elements in the presence of said sheet.

**BACKGROUND OF THE INVENTION**

It is well known in the art that the introduction of photographically useful compounds, such as photographic developers, couplers, development inhibitors, electron transfer agents, base precursors, fixing agents, i.e., ligand capable of binding silver, silver stabilizing agents and the like, into photographic elements can lead to premature reaction of the photographically useful compound with the other components of the photographic element. For example, placing conventional color developers, such as p-phenylenediamines and p-aminophenols, into sensitized photographic elements leads to desensitization of the silver halide emulsion and unsuitable fog. Much effort has therefore been directed at trying to produce effective blocked developers, which can be introduced in silver halide emulsion elements without deleterious desensitization or fog effects and which unblock chemically under conditions of development so that developer is free to participate in color forming (dye forming) reactions.

U.S. Pat. No. 3,342,599, to Reeves, discloses the use of Schiff base developer precursors. U.S. Pat. No. 4,157,915, to Hamaoka et al., and U.S. Pat. No. 4,060,418, to Waxman and Mourning, describe the preparation and use of carbamate blocked p-phenylenediamines. Color developing agents having  $\alpha$ -ketoacyl blocking groups are described in U.S. Pat. No 5,019,492.

All of these approaches and inventions have failed in practical product applications because of one or more of the following problems: desensitization of sensitized silver halide; unacceptably slow unblocking kinetics; instability of blocked developer yielding increased fog and/or decreased Dmax after storage; and the requirement of a dinucleophile, such as hydroxylamine, to initiate developer release.

The addition of a blocking group to a color developing agent results in an increase in molecular weight and generally results in a decrease in water solubility of the resulting blocked version of the parent color developing agent. As a result, the incorporation of these blocked developers in photographic elements is carried out using colloidal gelatin dispersions of the blocked developers. These dispersions are prepared using means well known in the art, wherein the developer precursor is dissolved in a high vapor pressure organic solvent (for example, ethyl acetate), along with, in some cases, a low vapor pressure organic solvent (such as dibutylphthalate), and then emulsified with an aqueous surfactant and gelatin solution. After emulsification, usually done with a colloid mill, the high vapor pressure organic solvent is removed by evaporation or by washing, as is well known in the art.

**PROBLEM TO BE SOLVED BY THE  
INVENTION**

There has been a need for a photographic element incorporating a photographically useful compound, such as a

developing agent, which is stable until development. Then, the element can be developed rapidly and easily. There has also been a need to simplify the preparation of the developer dispersion method and to eliminate the need for organic solvents in coating formulations. There has also been a need for a process for developing an image in a photographic element which employs a developing solution having a simplified composition.

**SUMMARY OF THE INVENTION**

These and other needs have been satisfied by providing a photographically useful reducing agent, such as a developer, in a sheet that can be brought into reactive association with an photographic element after said element has been imagewise exposed to light.

One aspect of this invention comprises a sheet comprising at least one photographically useful reducing agent ionically bound to an ion exchange matrix. In preferred embodiments of the invention, the sheet further comprises a binder and/or support and the ion exchange matrix comprises particles having an average particle size of less than about 10 micrometers ( $\mu\text{m}$ ).

The sheet can be prepared by any suitable process, for example the sheet can be formed of a solution of the ion exchange matrix in a solvent. In preferred embodiments of the invention, the ion exchange matrix is in the form of particles. To form the sheet a binder is added to the solution before casting. Suitable binders include, for example, cellulose derivatives (e.g., cellulose esters), gelatin (e.g., alkali-treated gelatin such as cattle bone or hide gelatin, or acid treated gelatin such as pigskin gelatin), deionized gelatin, gelatin derivatives (e.g., acetylated gelatin, phthalated gelatin, and the like) synthetic polymers, carriers, such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers, and the like. The amount of binder used is from about 1:3 to about 10: 1, based on the weight of the ion exchange matrix.

In preferred embodiment of the invention, a layer of binder plus ion exchange matrix is coated onto a support. Suitable supports include, for example, polymeric film, wood fiber, e.g., paper, metallic sheet and foil, glass and ceramic supporting elements. Preferred supports include, for example, polymeric film supports including films of cellulose nitrate and cellulose esters (such as cellulose triacetate and diacetate), polystyrene, polyamides, homo- and copolymers of vinyl chloride, poly(vinyl acetal), polycarbonate, homo- and copolymers of olefins such as polyethylene and polypropylene, and polyesters of dibasic aromatic carboxylic acids with divalent alcohols such as poly(ethylene terephthalate) or poly(ethylene naphthalate).

Another aspect of this invention comprises a method of processing a photographic element comprising at least one silver halide light-sensitive emulsion layer which comprises contacting the element with (a) a processing solution and (b) a sheet comprising a photographically useful reducing agent ionically bound to ion exchange matrix.

A further aspect of this invention comprises a method of processing a photographic element comprising at least one silver halide light-sensitive emulsion layer which comprises contacting the element with (a) a processing solution having a pH of about 8–13 and (b) a sheet comprising a photographically useful reducing agent ionically bound to an ionic exchange matrix.

A further aspect of this invention comprises a method of processing a photographic element comprising at least one silver halide light-sensitive emulsion layer which comprises contacting the element with (a) a processing solution having an ionic strength of greater than 0.001 M and (b) a sheet comprising a photographically useful reducing agent ionically bound to an ion exchange matrix.

Still another aspect of this invention comprises a method of processing a photographic element comprising at least one silver halide light-sensitive layer which comprises contacting the element with (a) a sheet comprising a photographically useful reducing agent ionically bound to an ion exchange matrix and (b) with thermal energy to elevate the temperature above 50° C.

Still a further aspect of this invention comprises a method of imaging comprising the steps of:

forming an image in an imagewise exposed light-sensitive silver halide element by one of the methods described above;

scanning said formed image to form a first electronic image representation from said formed image;

digitizing said first electronic image to form a digital image;

modifying said digital image to form a second electronic image representation; and

transforming, storing, transmitting, printing or displaying said second electronic image representation.

Yet a further aspect of this invention comprises a method of forming an image comprising the steps of:

forming an image in an imagewise exposed light-sensitive silver halide element by one of the methods described above;

scanning said formed image to form an electronic image representation from said formed image; and

transforming, storing, transmitting, printing or displaying said electronic image representation.

#### BRIEF DESCRIPTION OF THE DRAWINGS

FIG. 1 shows in block diagram form an apparatus for processing and viewing image formation obtained by scanning a photographic element of this invention.

FIG. 2 is a block diagram showing electronic signal processing of image bearing signals derived from scanning a developed color element according to the invention.

#### DETAILED DESCRIPTION OF THE INVENTION

The principles of ion exchange are well known and are described, for example, in *Chemical Engineer's Handbook*, Fifth Edition, Section 16. Ion exchange materials generally consist of a solid phase containing bound groups that carry an ionic charge, either positive or negative, in conjunction with free ions of opposite charge that can be displaced. Ion exchange materials have the characteristic of selectively taking up and storing one or more ionized solute species from a fluid phase. The concentration of bound ionic groups in the ion exchange material is called the stoichiometric capacity. The maximum uptake of a specific solute by the ion exchange resin is related to the stoichiometric capacity of the resin and to the adsorption strength of the solute to those bound groups. Ionic exchange resins useful in this invention include, for example, organic synthetic resins, inorganic resins and the like.

Cation-exchange resins generally contain bound sulfonic acid groups (for example,  $\text{SO}_3^-$ ). These resins are typically

commercially available in either the acidic form or the sodium form. Additionally, cation-exchange resins contain other bound acid groups such as carboxylic, phosphonic, phosphinic, (for example,  $\text{COO}^-$ ,  $\text{PO}_3^{2-}$ ,  $\text{HPO}_2^-$ ,  $\text{AsO}_2^-$ ,  $\text{SeO}_3^-$ , etc). Preferred cationic ion exchange resins are sulfonated copolymers derived from styrene and divinylbenzene with a sulfonation level of about 3 to about 5 meq/g.

Anionic-exchange resins involve quaternary ammonium groups (strongly basic) or other amino groups (weakly basic). Such resins preferably contain one or more of the following ionic groups:



Preferred anionic ion exchange resins are derived from copolymers of styrene and divinylbenzene contain at least one of the above ionic groups. A preferred anionic ion exchange resin comprises a copolymer derived from styrene and divinylbenzene containing trimethylbenzylammonium chloride groups.

Ion exchange reactions are reversible and involve chemically equivalent quantities. It is possible to recover the solute and to purify and reuse the ion exchange resin. In this case, conditions for regeneration must also exist. This can be accomplished with a solution containing the ion initially present in the solid. An ever-present excess of this ion during the regeneration step will cause the reaction equilibrium to reverse itself, restoring the resin to its initial condition.

For use in this invention, the ion exchange preferably comprises particles of about 0.01 to about 10 micrometers ( $\mu\text{m}$ ), more preferable about 0.05 to about 8  $\mu\text{m}$  and most preferably about 0.1 to about 5  $\mu\text{m}$ . Particles of the desired size can be prepared by standard techniques, such as milling, by preparing the particles by a limited coalescence procedure, or other procedures known in the art.

The photographic useful reducing agent is present in an amount of about 5 to about 100, preferably about 10 to about 90 and most preferably about 15 to about 90 mol percent of the ion exchange stoichiometric capacity of the ion exchange resin. The terms "acid" and "acidic", "base" and "basic" are used herein to refer to compounds known as Lewis acids and Lewis bases. Acids are molecules or ions capable of coordinating with unshared electron pairs and bases are molecules or ions which have such unshared electron pairs available for coordination. Lewis acids will coordinate with the anionic exchangers, and Lewis bases with the cation exchangers.

The photographically useful reducing agent can be, for example, a photographic developer, a blocked developer, a developer precursor, an electron transfer agent, a blocked electron transfer agent an electron transfer agent precursor or the like.

In a preferred embodiment of the invention, the photographically useful reducing agent is a developer. The developer can be an active developer or a blocked developer. A discussion of developers can be found in *Research Disclosure*, September 1996, Number 389, Item 38957 Section XIX, subsection A. September 1996, Number 389, Item 38957 (hereafter referred to as ("Research Disclosure I"). All sections referred to herein are sections of *Research Disclosure I*, unless otherwise indicated. (All Research Disclosures referenced herein are published by Kenneth Mason Publications, Ltd., Dudley Annex, 12a North Street,

Emsworth, Hampshire PO10 7DQ, ENGLAND). The developer can be organic or inorganic. Useful classes of organic developing agents include hydroquinones, catechols, aminophenols, pyrazolidones, phenylenediamines, tetrahydroquinolines, bis(pyridone)amines, cycloalkenones, pyrimidines, reductones and coumarins. Useful inorganic developing agents include compounds of a metal having at least two distinct valence states, which compounds are capable of reducing ionic silver to metallic silver. Such metals include iron, titanium, vanadium and chromium, and the metal compounds employed are typically complexes with organic compounds such as polycarboxylic acids or aminopolycarboxylic acids.

Included among useful developing agents are the iodohydroquinones of Duennebier et al U.S. Pat. No. 3,297,445, the aminohydroxy cycloalkenones of Gabrielsen et al U.S. Pat. No. 3,690,872, the 5-hydroxy and 5-aminopyrimidines of Wyand et al U.S. Pat. No. 3,672,891, the N-acyl derivatives of p-aminophenols of Porter et al U.K. Patent 1,045,303, the 3-pyrazolidones of Kendall U.S. Pat. No. 2,289,367, Allen U.S. Pat. No. 2,772,282, Ishikawa et al U.S. Pat. No. 4,845,016 Stewart et al U.K. Patent 1,023,701 and DeMarle et al U.S. Pat. Nos. 3,221,023 and 3,241,967, the anhydriodihydro reductones of Gabrielsen et al U.S. Pat. No. 3,672,896, the heterocyclic-sulfonhydrazides of Clarke et al EPO 0 545 491, the N-(4-aminophenyl)pyrrolidine derivatives of Ohki et al U.S. Pat. No. 5,278,034, the 6-aminotetrahydroquinolines of Taniguchi et al EPO 0 670 312, the heterocyclic compounds of Hagemann DE 4,241,532, and the 6-hydroxy and 6-aminocoumarins of Oftedahl U.S. Pat. No. 3,615,521. Particularly useful primary aromatic amino color developing agents are the p-phenylenediamines and especially the N-N-dialkyl-p-phenylenediamines in which the alkyl groups or the aromatic nucleus can be substituted or unsubstituted. Common p-phenylenediamine color developing agents are N,N-diethyl-p-phenylenediamine monohydrochloride, 4-N,N-diethyl-2-methylphenylenediamine monohydrochloride, 4-(N-ethyl-N-2-methanesulfonylaminoethyl)-2-methylphenylenediamine sesquisulfate monohydrate, and 4-(N-ethyl-N-2-hydroxyethyl)-2-methylphenylenediamine sulfate. Other p-phenylenediamines, similar compounds, and their use include those described in Nakamura et al U.S. Pat. No. 5,427,897, Miyayashi et al U.S. Pat. No. 5,380,625, Hajima et al U.S. Pat. No. 5,328,812, Taniguchi et al U.S. Pat. No. 5,264,331, Kuse et al U.S. Pat. No. 5,202,229, Mikoshiba et al U.S. Pat. No. 5,223,380, Nakamura et al U.S. Pat. No. 5,176,987, Yoshizawa et al U.S. Pat. No. 5,006,437, Nakamura U.S. Pat. No. 5,102,778 and Nakagawa et al U.S. Pat. No. 5,043,254. Advantageous results can be obtained with combinations of organic and inorganic developing agents as described in Vought *Research Disclosure*, Vol. 150, October, 1976, Item 15034, and with combinations of different types of organic developing agents such as the combination of anhydriodihydroamino reductones and aminomethyl hydroquinones of Youngquist U.S. Pat. No. 3,666,457, the combination of a color developer and a 3-pyrazolidone of Twist WO 92/10789 and the combination of ascorbic acid and 3-pyrazolidone of Suthers U.K. Patent 1,281,516. Developing agents can be incorporated in photographic processing elements in the form of precursors. Examples of such precursors include the halogenated acyl hydroquinones of Porter et al U.S. Pat. No. 3,246,988, the N-acyl derivatives of aminophenols of Porter et al U.S. Pat. No. 3,291,609, the reaction products of a catechol or hydroquinone with a metal described in Barr U.S. Pat. No. 3,295,978, the quinhydrone dyes of Haefner et al U.S. Pat.

No. 3,565,627, the cyclohex-2-ene-1,4-diones and cyclohex-2-ene-1-one-4-monoketals of Chapman et al U.S. Pat. No. 3,586,506, the Schiff bases of p-phenylenediamines of Pupo et al *Research Disclosure*, Vol. 151, November, 1976, Item 15159 and the blocked developers of Southby et al U.S. Pat. No. 5,256,525. The developing agent can be added to the layer in the form of a dispersion with a film-forming polymer in a water-immiscible solvent as illustrated by Dunn et al U.S. Pat. No. 3,518,088, as a dispersion with a polymer latex as illustrated by Chen *Research Disclosure*, Vol. 159, July, 1977, Item 15930, and Pupo et al *Research Disclosure*, Vol. 148, August, 1976, Item 14850, or as a solid particle dispersion as described by Texter et al U.S. Pat. No. 5,240,821. Incorporated primary amine color developing agents or precursors therefore are also used in photographic elements that are processed in low volumes of processing solutions as described by Texter et al U.S. Pat. No. 5,411,840.

Preferred developers include aminophenols, phenylenediamines, hydroquinones and pyrazolidones. Representative patents describing such developing agents are U.S. Pat. Nos. 2,193,015; 2,108,243; 2,592,364; 3,656,950; 3,658,525; 2,751,297; 2,289,367; 2,772,282; 2,743,279; 2,753,256; and 2,304,953.

Structures of preferred developing agents are:



wherein R<sub>1</sub> is hydrogen, halogen (e.g. chloro, bromo), alkyl or alkoxy (preferably of 1 to 4 carbon atoms); R<sub>2</sub> is hydrogen or alkyl (preferably of 1 to 4 carbon atoms); R<sub>3</sub> is hydrogen, alkyl, alkoxy or alkenedioxy (preferably of 1 to 4 carbon atoms); and R<sub>4</sub>, R<sub>5</sub>, R<sub>6</sub>, R<sub>7</sub> and R<sub>8</sub> are individually hydrogen, alkyl, hydroxyalkyl or sulfoalkyl (preferably of 1 to 4 carbon atoms).

Particularly preferred developers are, p-phenylenediamines or p-aminophenols. Especially preferred are p-phenylenediamines.

In other embodiments of the invention the photographically useful reducing agent is an electron transfer agent, blocked electron transfer agent or electron transfer agent precursor.

The term "electron transfer agent" or ETA is employed in its art recognized sense of denoting a silver halide developing agent that donates an electron (becomes oxidized) in

reducing  $\text{Ag}^+$  in silver halide to silver  $\text{Ag}^0$  and is then regenerated to its original non-oxidized state by entering into a redox reaction with primary amine color developing agent. In the redox reaction the color developing agent is oxidized and hence activated for coupling.

Preferred electron transfer agents 1-aryl-3-pyrazolidinone derivatives, a hydroquinone or derivative thereof, a catechol or derivative thereof, or an acylhydrazine or derivative thereof. The electron transfer agent pyrazolidinone moieties which have been found to be useful in providing development acceleration function are derived from compounds generally of the type described in U.S. Pat. Nos. 4,209,580; 4,463,081; 4,471,045; and 4,481,287, the entire disclosures of which are incorporated herein by reference, and in published Japanese patent application No. 62-123,172. Such compounds comprise a 3-pyrazolidinone structure having an unsubstituted or substituted aryl group in the 1-position. Preferably these compounds have one or more alkyl groups in the 4 or 5-positions of the pyrazolidinone ring. Particularly useful electron transfer agents are described in Platt et al U.S. Pat. No. 4,912,025, and Michno et al U.S. Pat. No. 4,859,578, the entire disclosures of which are incorporated herein by reference.

The sheet containing an ion exchanged reducing agent can be used during the processing of a photographic element in any form as discussed more fully below during Type I, Type II or Type III processing. For the purpose of the following discussion, the processing sheet of the current invention will be referred to as the photographic processing element, and the light sensitive emulsion containing material for use with the present invention will be referred to as the photographic element. The emulsion layer for use with the photographic processing element can comprise any one or more of the light sensitive layers of the photographic element. The photographic elements can be black and white elements, single color elements or multicolor elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like. All of these can be coated on a support which can be transparent or reflective (for example, a paper support).

Photographic elements for use with the present invention may also usefully include a magnetic recording material as described in *Research Disclosure*, Item 34390, November 1992, or a transparent magnetic recording layer such as a layer containing magnetic particles on the underside of a transparent support as in U.S. Pat. Nos. 4,279,945 and 4,302,523. The element typically will have a total thickness (excluding the support) of from 5 to 30 microns. While the

order of the color sensitive layers can be varied, they will normally be red-sensitive, green-sensitive and blue-sensitive, in that order on a transparent support, (that is, blue sensitive furthest from the support) and the reverse order on a reflective support being typical.

The present invention also contemplates the use of photographic elements for use with the present invention in what are often referred to as single use cameras (or "film with lens" units). These cameras are sold with film pre-loaded in them and the entire camera is returned to a processor with the exposed film remaining inside the camera. Such cameras may have glass or plastic lenses through which the photographic element is exposed.

In the following discussion of suitable materials for use in elements of this invention, reference will be made to *Research Disclosure*, September 1996, Number 389, Item 38957, which will be identified hereafter by the term "Research Disclosure I." The Sections hereafter referred to are Sections of the Research Disclosure I unless otherwise indicated. All Research Disclosures referenced are published by Kenneth Mason Publications, Ltd., Dudley Annex, 12a North Street, Emsworth, Hampshire PO10 7DQ, ENGLAND. The foregoing references and all other references cited in this application, are incorporated herein by reference.

The silver halide emulsions employed in the photographic elements for use with the present invention may be negative-working, such as surface-sensitive emulsions or unfogged internal latent image forming emulsions, or positive working emulsions of the internal latent image forming type (that are fogged during processing). Suitable emulsions and their preparation as well as methods of chemical and spectral sensitization are described in Sections I through V. Color materials and development modifiers are described in Sections V through XX. Vehicles which can be used in the photographic elements and photographic processing elements are described in Section II, and various additives such as brighteners, antifoggants, stabilizers, light absorbing and scattering materials, hardeners, coating aids, plasticizers, lubricants and matting agents are described, for example, in Sections VI through XIII. Manufacturing methods are described in all of the sections, layer arrangements particularly in Section XI, exposure alternatives in Section XVI, and processing methods and agents in Sections XIX and XX.

With negative working silver halide a negative image can be formed. Optionally a positive (or reversal) image can be formed although a negative image is typically first formed.

The photographic elements may also use colored couplers (e.g. to adjust levels of interlayer correction) and masking couplers such as those described in EP 213 490; Japanese Published Application 58-172,647; U.S. Pat. No. 2,983,608; German Application DE 2,706,117C; U.K. Patent 1,530,272; Japanese Application A-113935; U.S. Pat. No. 4,070,191 and German Application DE 2,643,965. The masking couplers may be shifted or blocked.

The photographic elements may also contain materials that accelerate or otherwise modify the processing steps of bleaching or fixing to improve the quality of the image. Bleach accelerators described in EP 193 389; EP 301 477; U.S. Pat. Nos. 4,163,669; 4,865,956; and 4,923,784 are particularly useful. Also contemplated is the use of nucleating agents, development accelerators or their precursors (UK Patent 2,097,140; U.K. Patent 2,131,188); development inhibitors and their precursors (U.S. Pat. No. 5,460,932; 5,478,711); electron transfer agents (U.S. Pat. No. 4,859,578; 4,912,025); antifogging and anti color-mixing agents such as derivatives of hydroquinones, aminophenols,

amines, gallic acid; catechol; ascorbic acid; hydrazides; sulfonamidophenols; and non color-forming couplers.

The photographic elements may also contain filter dye layers comprising colloidal silver sol or yellow and/or magenta filter dyes and/or antihalation dyes (particularly in an undercoat beneath all light sensitive layers or in the side of the support opposite that on which all light sensitive layers are located) either as oil-in-water dispersions, latex dispersions or as solid particle dispersions. Additionally, they may be used with "smearing" couplers (e.g. as described in U.S. Pat. No. 4,366,237; EP 096 570; U.S. Pat. Nos. 4,420,556; and 4,543,323.) Also, the couplers may be blocked or coated in protected form as described, for example, in Japanese Application 61/258,249 or U.S. Pat. No. 5,019,492.

The photographic elements may further contain other image-modifying compounds such as "Development Inhibitor-Releasing" compounds (DIR's). Useful additional DIR's for elements of the present invention, are known in the art and examples are described in U.S. Pat. Nos. 3,137, 578; 3,148,022; 3,148,062; 3,227,554; 3,384,657; 3,379, 529; 3,615,506; 3,617,291; 3,620,746; 3,701,783; 3,733, 201; 4,049,455; 4,095,984; 4,126,459; 4,149,886; 4,150, 228; 4,211,562; 4,248,962; 4,259,437; 4,362,878; 4,409, 323; 4,477,563; 4,782,012; 4,962,018; 4,500,634; 4,579, 816; 4,607,004; 4,618,571; 4,678,739; 4,746,600; 4,746, 601; 4,791,049; 4,857,447; 4,865,959; 4,880,342; 4,886, 736; 4,937,179; 4,946,767; 4,948,716; 4,952,485; 4,956, 269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

DIR compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969), incorporated herein by reference.

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO101 7DQ, England, incorporated herein by reference. The emulsions and materials to form elements of the present invention, may be coated on pH adjusted support as described in U.S. Pat. No. 4,917,994; with epoxy solvents (EP 0 164 961); with additional stabilizers (as described, for example, in U.S. Pat. Nos. 4,346,165; 4,540,653 and 4,906, 559); with ballasted chelating agents such as those in U.S. Pat. No. 4,994,359 to reduce sensitivity to polyvalent cations such as calcium; and with stain reducing compounds such as described in U.S. Pat. No. 5,068,171 and U.S. Pat. No. 5,096,805. Other compounds which may be useful in photographic elements are disclosed in Japanese Published Applications 83-09,959; 83-62,586; 90-072,629; 90-072, 630; 90-072,632; 90-072,633; 90-072,634; 90-077,822; 90-078,229; 90-078,230; 90-079,336; 90-079,338; 90-079, 690; 90-079,691; 90-080,487; 90-080,489; 90-080,490; 90080,491; 90-080,492; 90-080,494; 90-085,928; 90-086, 669; 90-086,670; 90-087,361; 90-087,362; 90-087,363; 90-087,364; 90-088,096; 90-088,097; 90-093,662; 90-093, 663; 90-093,664; 90-093,665; 90-093,666; 90-093,668; 90-094,055; 90-094,056; 90-101,937; 90-103,409; 90-151, 577.

The silver halide used in the photographic elements may be silver iodobromide, silver bromide, silver chloride, silver chlorobromide, silver chloroiodobromide, and the like.

The type of silver halide grains preferably include polymorphic, cubic, and octahedral. The grain size of the silver halide may have any distribution known to be useful in photographic compositions, and may be either polydispersed or monodispersed.

Tabular grain silver halide emulsions may also be used.

Tabular grains are those with two parallel major faces each clearly larger than any remaining grain face and tabular grain emulsions are those in which the tabular grains account for at least 30 percent, more typically at least 50 percent, preferably >70 percent and optimally >90 percent of total grain projected area. The tabular grains can account for substantially all (>97 percent) of total grain projected area. The tabular grain emulsions can be high aspect ratio tabular grain emulsions—i.e.,  $ECD/t > 8$ , where ECD is the diameter of a circle having an area equal to grain projected area and t is tabular grain thickness; intermediate aspect ratio tabular grain emulsions—i.e.,  $ECD/t = 5$  to 8; or low aspect ratio tabular grain emulsions—i.e.,  $ECD/t = 2$  to 5. The emulsions typically exhibit high tabularity (T), where T (i.e.,  $ECD/t^2$ ) >25 and ECD and t are both measured in micrometers ( $\mu m$ ). The tabular grains can be of any thickness compatible with achieving an aim average aspect ratio and/or average tabularity of the tabular grain emulsion. Preferably the tabular grains satisfying projected area requirements are those having thicknesses of <0.3  $\mu m$ , thin (<0.2  $\mu m$ ) tabular grains being specifically preferred and ultrathin (<0.07  $\mu m$ ) tabular grains being contemplated for maximum tabular grain performance enhancements. When the native blue absorption of iodohalide tabular grains is relied upon for blue speed, thicker tabular grains, typically up to 0.5  $\mu m$  in thickness, are contemplated.

High iodide tabular grain emulsions are illustrated by House U.S. Pat. No. 4,490,458, Maskasky U.S. Pat. No. 4,459,353 and Yagi et al EPO 0 410 410.

Tabular grains formed of silver halide(s) that form a face centered cubic (rock salt type) crystal lattice structure can have either {100} or {111} major faces. Emulsions containing {111} major face tabular grains, including those with controlled grain dispersities, halide distributions, twin plane spacing, edge structures and grain dislocations as well as adsorbed {111} grain face stabilizers, are illustrated in those references cited in *Research Disclosure I*, Section I.B.(3) (page 503).

The silver halide grains to be used in the invention may be prepared according to methods known in the art, such as those described in *Research Disclosure I* and James, *The Theory of the Photographic Process*. These include methods such as ammoniacal emulsion making, neutral or acidic emulsion making, and others known in the art. These methods generally involve mixing a water soluble silver salt with a water soluble halide salt in the presence of a protective colloid, and controlling the temperature, pAg, pH values, etc, at suitable values during formation of the silver halide by precipitation.

In the course of grain precipitation one or more dopants (grain occlusions other than silver and halide) can be introduced to modify grain properties. For example, any of the various conventional dopants disclosed in *Research Disclosure*, Item 38957, Section I. Emulsion grains and their preparation, sub-section G. Grain modifying conditions and adjustments, paragraphs (3), (4) and (5), can be present in the emulsions used. In addition it is specifically contemplated to dope the grains with transition metal hexaco-

ordination complexes containing one or more organic ligands, as taught by Olm et al U.S. Pat. No. 5,360,712, the disclosure of which is here incorporated by reference.

It is specifically contemplated to incorporate in the face centered cubic crystal lattice of the grains a dopant capable of increasing imaging speed by forming a shallow electron trap (hereinafter also referred to as a SET) as discussed in Research Disclosure Item 36736 published November 1994, here incorporated by reference.

The SET dopants are effective at any location within the grains. Generally better results are obtained when the SET dopant is incorporated in the exterior 50 percent of the grain, based on silver. An optimum grain region for SET incorporation is that formed by silver ranging from 50 to 85 percent of total silver forming the grains. The SET can be introduced all at once or run into the reaction vessel over a period of time while grain precipitation is continuing. Generally SET forming dopants are contemplated to be incorporated in concentrations of at least  $1 \times 10^{-7}$  mole per silver mole up to their solubility limit, typically up to about  $5 \times 10^{-4}$  mole per silver mole.

SET dopants are known to be effective to reduce reciprocity failure. In particular the use of iridium hexacoordination complexes or  $\text{Ir}^{+4}$  complexes as SET dopants is advantageous.

Iridium dopants that are ineffective to provide shallow electron traps (non-SET dopants) can also be incorporated into the grains of the silver halide grain emulsions to reduce reciprocity failure.

To be effective for reciprocity improvement the Ir can be present at any location within the grain structure. A preferred location within the grain structure for Ir dopants to produce reciprocity improvement is in the region of the grains formed after the first 60 percent and before the final 1 percent (most preferably before the final 3 percent) of total silver forming the grains has been precipitated. The dopant can be introduced all at once or run into the reaction vessel over a period of time while grain precipitation is continuing. Generally reciprocity improving non-SET Ir dopants are contemplated to be incorporated at their lowest effective concentrations.

The contrast of the photographic element can be further increased by doping the grains with a hexacoordination complex containing a nitrosyl or thionitrosyl ligand (NZ dopants) as disclosed in McDugle et al U.S. Pat. No. 4,933,272, the disclosure of which is here incorporated by reference.

The contrast increasing dopants can be incorporated in the grain structure at any convenient location. However, if the NZ dopant is present at the surface of the grain, it can reduce the sensitivity of the grains. It is therefore preferred that the NZ dopants be located in the grain so that they are separated from the grain surface by at least 1 percent (most preferably at least 3 percent) of the total silver precipitated in forming the silver iodochloride grains. Preferred contrast enhancing concentrations of the NZ dopants range from  $1 \times 10^{-11}$  to  $4 \times 10^{-8}$  mole per silver mole, with specifically preferred concentrations being in the range from  $10^{-10}$  to  $10^{-8}$  mole per silver mole.

Although generally preferred concentration ranges for the various SET, non-SET Ir and NZ dopants have been set out above, it is recognized that specific optimum concentration ranges within these general ranges can be identified for specific applications by routine testing. It is specifically contemplated to employ the SET, non-SET Ir and NZ dopants singly or in combination. For example, grains containing a combination of an SET dopant and a non-SET

Ir dopant are specifically contemplated. Similarly SET and NZ dopants can be employed in combination. Also NZ and Ir dopants that are not SET dopants can be employed in combination. Finally, the combination of a non-SET Ir dopant with a SET dopant and an NZ dopant. For this latter three-way combination of dopants it is generally most convenient in terms of precipitation to incorporate the NZ dopant first, followed by the SET dopant, with the non-SET Ir dopant incorporated last.

The photographic processing elements of the present invention generally include a vehicle for coating the ion exchange particles. Useful vehicles include both naturally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), deionized gelatin, gelatin derivatives (e.g., acetylated gelatin, phthalated gelatin, and the like), and others as described in *Research Disclosure I*. Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers, and the like, as described in *Research Disclosure I*. The vehicle can also include any of the addenda known to be useful in photographic emulsions.

The silver halide to be used with the invention may be advantageously subjected to chemical sensitization. Compounds and techniques useful for chemical sensitization of silver halide are known in the art and described in *Research Disclosure I* and the references cited therein. Compounds useful as chemical sensitizers, include, for example, active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 4 to 8, and temperatures of from 30 to 80° C., as described in *Research Disclosure I*, Section IV (pages 510-511) and the references cited therein.

The silver halide may be sensitized by sensitizing dyes by any method known in the art, such as described in *Research Disclosure I*. The dye may be added to an emulsion of the silver halide grains and a hydrophilic colloid at any time prior to (e.g., during or after chemical sensitization) or simultaneous with the coating of the emulsion on a photographic element. The dyes may, for example, be added as a solution in water or an alcohol. The dye/silver halide emulsion may be mixed with a dispersion of color image-forming coupler immediately before coating or in advance of coating (for example, 2 hours).

Photographic elements for use with the present invention are preferably imagewise exposed using any of the known techniques, including those described in *Research Disclosure I*, section XVI. This typically involves exposure to light in the visible region of the spectrum, and typically such exposure is of a live image through a lens, although exposure can also be exposure to a stored image (such as a computer stored image) by means of light emitting devices (such as light emitting diodes, CRT and the like).

In a preferred embodiment the photographic element for use with the invention is a color negative film. Prints can be made from the film by conventional optical techniques or by scanning the film and printing using a laser, light emitting diode, cathode ray tube or the like.

A typical color negative film construction useful in the practice of the invention is illustrated by the following element, SCN-1:

| Element SCN-1 |                            |
|---------------|----------------------------|
| SOC           | Surface Overcoat           |
| BU            | Blue Recording Layer Unit  |
| IL1           | First Interlayer           |
| GU            | Green Recording Layer Unit |
| IL2           | Second Interlayer          |
| RU            | Red Recording Layer Unit   |
| AHU           | Antihalation Layer Unit    |
| S             | Support                    |
| SOC           | Surface Overcoat           |

The support S can be either reflective or transparent, which is usually preferred. When reflective, the support is white and can take the form of any conventional support currently employed in color print elements. When the support is transparent, it can be colorless or tinted and can take the form of any conventional support currently employed in color negative elements—e.g., a colorless or tinted transparent film support. Details of support construction are well understood in the art. Examples of useful supports are poly(vinyl acetal) film, polystyrene film, poly(ethyleneterephthalate) film, poly(ethylene naphthalate) film, polycarbonate film, and related films and resinous materials, as well as paper, cloth, glass, metal, and other supports that withstand the anticipated processing conditions. The element can contain additional layers, such as filter layers, interlayers, overcoat layers, subbing layers, antihalation layers and the like. Transparent and reflective support constructions, including subbing layers to enhance adhesion, are disclosed in Section XV Supports of *Research Disclosure I*.

Each of blue, green and red recording layer units BU, GU and RU are formed of one or more hydrophilic colloid layers and contain at least one radiation-sensitive silver halide emulsion and coupler, including at least one dye image-forming coupler. It is preferred that the green, and red recording units are subdivided into at least two recording layer sub-units to provide increased recording latitude and reduced image granularity. In the simplest contemplated construction each of the layer units or layer sub-units consists of a single hydrophilic colloid layer containing emulsion and coupler. When coupler present in a layer unit or layer sub-unit is coated in a hydrophilic colloid layer other than an emulsion containing layer, the coupler containing hydrophilic colloid layer is positioned to receive oxidized color developing agent from the emulsion during development. Usually the coupler containing layer is the next adjacent hydrophilic colloid layer to the emulsion containing layer.

In order to ensure excellent image sharpness, and to facilitate manufacture and use in cameras, all of the sensitized layers are preferably positioned on a common face of the support. When in spool form, the element will be spooled such that when unspooled in a camera, exposing light strikes all of the sensitized layers before striking the face of the support carrying these layers. Further, to ensure excellent sharpness of images exposed onto the element, the total thickness of the layer units above the support should be controlled. Generally, the total thickness of the sensitized layers, interlayers and protective layers on the exposure face of the support are less than about 35  $\mu\text{m}$  and preferably less than about 25  $\mu\text{m}$  and most preferably less than about 20  $\mu\text{m}$ .

Any convenient selection from among conventional radiation-sensitive silver halide emulsions can be incorporated within the layer units and used to provide the spectral absorptances desired. Most commonly high bromide or high chloride emulsions containing a minor amount of iodide are employed. To realize higher rates of processing, high chloride emulsions can be employed. Radiation-sensitive silver chloride, silver bromide, silver iodobromide, silver iodochloride, silver chlorobromide, silver bromochloride, silver iodochlorobromide and silver iodobromochloride grains are all contemplated. The grains can be either regular or irregular (e.g., tabular). Tabular grain emulsions, those in which tabular grains account for at least 50 (preferably at least 70 and optimally at least 90) percent of total grain projected area are particularly advantageous for increasing speed in relation to granularity. To be considered tabular a grain requires two major parallel faces with a ratio of its equivalent circular diameter (ECD) to its thickness of at least 2. Further, the tabular grains can have either {111} or {100} major faces. Specifically preferred tabular grain emulsions are those having a tabular grain average aspect ratio of at least 5 and, optimally, greater than 8. Preferred mean tabular grain thicknesses are less than 0.3  $\mu\text{m}$  (most preferably less than 0.2  $\mu\text{m}$ ). Ultrathin tabular grain emulsions, those with mean tabular grain thicknesses of less than 0.07  $\mu\text{m}$ , are specifically contemplated. The grains preferably form surface latent images so that they produce negative images when processed in a surface developer in color negative film forms of the invention.

Illustrations of conventional radiation-sensitive silver halide emulsions are provided by *Research Disclosure*, Item 38957, cited above, I. Emulsion grains and their preparation. Chemical sensitization of the emulsions, which can take any conventional form, is illustrated in section IV. Chemical sensitization. Compounds useful as chemical sensitizers, include, for example, active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 4 to 8, and temperatures of from 30 to 80°C. Spectral sensitization and sensitizing dyes, which can take any conventional form, are illustrated by section V. Spectral sensitization and desensitization. The dye may be added to an emulsion of the silver halide grains and a hydrophilic colloid at any time prior to (e.g., during or after chemical sensitization) or simultaneous with the coating of the emulsion on a photographic element. The dyes may, for example, be added as a solution in water or an alcohol or as a dispersion of solid particles. The emulsion layers also typically include one or more antifoggants or stabilizers, which can take any conventional form, as illustrated by section VII. Antifoggants and stabilizers.

While any useful quantity of light-sensitive silver, as silver halide, can be employed in the elements useful in this invention, it is preferred that the total quantity be less than 10 g/m<sup>2</sup> of silver. Silver quantities of less than 7 g/m<sup>2</sup> are preferred, and silver quantities of less than 5 g/m<sup>2</sup> are even more preferred. The lower quantities of silver improve the optics of the elements, thus enabling the production of sharper pictures using the elements. These lower quantities of silver are additionally important in that they enable rapid development and desilvering of the elements. Conversely, a silver coating coverage of at least 1.5 g of coated silver per m<sup>2</sup> of support surface area in the element is preferred so as to realize an exposure latitude of at least 2.7 log E while maintaining an adequately low graininess position for pictures intended to be enlarged. For color display elements, substantially lower silver coating coverages are typically employed.

BU contains at least one yellow dye image-forming coupler, GU contains at least one magenta dye image-forming coupler, and RU contains at least one cyan dye image-forming coupler. Any convenient combination of conventional dye image-forming couplers can be employed. Conventional dye image-forming couplers are illustrated by *Research Disclosure*, Item 38957, cited above, X. Dye image formers and modifiers, B. Image-dye-forming couplers.

It is common practice to coat one, two or three separate emulsion layers within a single dye image-forming layer unit. When two or more emulsion layers are coated in a single layer unit, they are typically chosen to differ in sensitivity. When a more sensitive emulsion is coated over a less sensitive emulsion, a higher speed is realized than when the two emulsions are blended. When a less sensitive emulsion is coated over a more sensitive emulsion, a higher contrast is realized than when the two emulsions are blended. It is preferred that the most sensitive emulsion be located nearest the source of exposing radiation and the slowest emulsion be located nearest the support.

One or more of the layer units is preferably subdivided into at least two, and more preferably three or more sub-unit layers. It is preferred that all light-sensitive silver halide emulsions in the color recording unit have spectral sensitivity in the same region of the visible spectrum. In this embodiment, while all silver halide emulsions incorporated in the unit have spectral absorptance according to invention, it is expected that there are minor differences in spectral absorptance properties between them. In still more preferred embodiments, the sensitizations of the slower silver halide emulsions are specifically tailored to account for the light shielding effects of the faster silver halide emulsions of the layer unit that reside above them, in order to provide an imagewise uniform spectral response by the photographic recording material as exposure varies with low to high light levels. Thus higher proportions of peak light absorbing spectral sensitizing dyes may be desirable in the slower emulsions of the subdivided layer unit to account for on-peak shielding and broadening of the underlying layer spectral sensitivity.

The interlayers IL1 and IL2 are hydrophilic colloid layers having as their primary function color contamination reduction—i.e., prevention of oxidized developing agent from migrating to an adjacent recording layer unit before reacting with dye-forming coupler. The interlayers are in part effective simply by increasing the diffusion path length that oxidized developing agent must travel. To increase the effectiveness of the interlayers to intercept oxidized developing agent, it is conventional practice to incorporate oxidized developing agent. Antistain agents (oxidized developing agent scavengers) can be selected from among those disclosed by *Research Disclosure*, Item 38957, X. Dye image formers and modifiers, D. Hue modifiers/stabilization, paragraph (2). When one or more silver halide emulsions in GU and RU are high bromide emulsions and, hence have significant native sensitivity to blue light, it is preferred to incorporate a yellow filter, such as Carey Lea silver or a yellow processing solution decolorizable dye, in IL1. Suitable yellow filter dyes can be selected from among those illustrated by *Research Disclosure*, Item 38957, VIII. Absorbing and scattering materials, B. Absorbing materials.

The antihalation layer unit AHU typically contains a processing solution removable or decolorizable light absorbing material, such as one or a combination of pigments and dyes. Suitable materials can be selected from among those disclosed in *Research Disclosure*, Item 38957, VIII. Absorb-

ing materials. A common alternative location for AHU is between the support S and the recording layer unit coated nearest the support.

The surface overcoats SOC are hydrophilic colloid layers that are provided for physical protection of the color negative elements during handling and processing. Each SOC also provides a convenient location for incorporation of addenda that are most effective at or near the surface of the color negative element. In some instances the surface overcoat is divided into a surface layer and an interlayer, the latter functioning as spacer between the addenda in the surface layer and the adjacent recording layer unit. In another common variant form, addenda are distributed between the surface layer and the interlayer, with the latter containing addenda that are compatible with the adjacent recording layer unit. Most typically the SOC contains addenda, such as coating aids, plasticizers and lubricants, antistats and matting agents, such as illustrated by *Research Disclosure*, Item 38957, IX. Coating physical property modifying addenda. The SOC overlying the emulsion layers additionally preferably contains an ultraviolet absorber, such as illustrated by *Research Disclosure*, Item 38957, VI. UV dyes/optical brighteners/luminescent dyes, paragraph (1). In like manner, similar overcoats can be coated in conjunction with the photographic processing elements of this invention comprising photographically useful reducing agent ionically bound to an ion exchange matrix.

Instead of the layer unit sequence of element SCN-1, alternative layer units sequences can be employed and are particularly attractive for some emulsion choices. Using high chloride emulsions and/or thin (<0.2  $\mu\text{m}$  mean grain thickness) tabular grain emulsions all possible interchanges of the positions of BU, GU and RU can be undertaken without risk of blue light contamination of the minus blue records, since these emulsions exhibit negligible native sensitivity in the visible spectrum. For the same reason, it is unnecessary to incorporate blue light absorbers in the interlayers.

When the emulsion layers within a dye image-forming layer unit differ in speed, it is conventional practice to limit the incorporation of dye image-forming coupler in the layer of highest speed to less than a stoichiometric amount, based on silver. The function of the highest speed emulsion layer is to create the portion of the characteristic curve just above the minimum density—i.e., in an exposure region that is below the threshold sensitivity of the remaining emulsion layer or layers in the layer unit. In this way, adding the increased granularity of the highest sensitivity speed emulsion layer to the dye image record produced is minimized without sacrificing imaging speed.

In the foregoing discussion the blue, green and red recording layer units are described as containing yellow, magenta and cyan image dye-forming couplers, respectively, as is conventional practice in color negative elements used for printing. The invention can be suitably applied to conventional color negative construction as illustrated. Color reversal film construction would take a similar form, with the exception that colored masking couplers would be completely absent; in typical forms, development inhibitor releasing couplers would also be absent. In preferred embodiments, the color negative elements are intended exclusively for scanning to produce three separate electronic color records. Thus the actual hue of the image dye produced is of no importance. What is essential is merely that the dye image produced in each of the layer units be differentiable from that produced by each of the remaining layer units. To provide this capability of differentiation

it is contemplated that each of the layer units contain one or more dye image-forming couplers chosen to produce image dye having an absorption half-peak bandwidth lying in a different spectral region. It is immaterial whether the blue, green or red recording layer unit forms a yellow, magenta or cyan dye having an absorption half peak bandwidth in the blue, green or red region of the spectrum, as is conventional in a color negative element intended for use in printing, or an absorption half-peak bandwidth in any other convenient region of the spectrum, ranging from the near ultraviolet (300-400 nm) through the visible and through the near infrared (700-1200 nm), so long as the absorption half-peak bandwidths of the image dye in the layer units extend over substantially non-coextensive wavelength ranges. The term "substantially non-coextensive wavelength ranges" means that each image dye exhibits an absorption half-peak band width that extends over at least a 25 (preferably 50) nm spectral region that is not occupied by an absorption half-peak band width of another image dye. Ideally the image dyes exhibit absorption half-peak band widths that are mutually exclusive.

When a layer unit contains two or more emulsion layers differing in speed, it is possible to lower image granularity in the image to be viewed, recreated from an electronic record, by forming in each emulsion layer of the layer unit a dye image which exhibits an absorption half-peak band width that lies in a different spectral region than the dye images of the other emulsion layers of layer unit. This technique is particularly well suited to elements in which the layer units are divided into sub-units that differ in speed. This allows multiple electronic records to be created for each layer unit, corresponding to the differing dye images formed by the emulsion layers of the same spectral sensitivity. The digital record formed by scanning the dye image formed by an emulsion layer of the highest speed is used to recreate the portion of the dye image to be viewed lying just above minimum density. At higher exposure levels second and, optionally, third electronic records can be formed by scanning spectrally differentiated dye images formed by the remaining emulsion layer or layers. These digital records contain less noise (lower granularity) and can be used in recreating the image to be viewed over exposure ranges above the threshold exposure level of the slower emulsion layers. This technique for lowering granularity is disclosed in greater detail by Sutton U.S. Pat. No. 5,314,794, the disclosure of which is here incorporated by reference.

Each layer unit of the color negative elements useful in the invention produces a dye image characteristic curve gamma of less than 1.5, which facilitates obtaining an exposure latitude of at least 2.7 log E. A minimum acceptable exposure latitude of a multicolor photographic element is that which allows accurately recording the most extreme whites (e.g., a bride's wedding gown) and the most extreme blacks (e.g., a bride groom's tuxedo) that are likely to arise in photographic use. An exposure latitude of 2.6 log E can just accommodate the typical bride and groom wedding scene. An exposure latitude of at least 3.0 log E is preferred, since this allows for a comfortable margin of error in exposure level selection by a photographer. Even larger exposure latitudes are specifically preferred, since the ability to obtain accurate image reproduction with larger exposure errors is realized. Whereas in color negative elements intended for printing, the visual attractiveness of the printed scene is often lost when gamma is exceptionally low, when color negative elements are scanned to create digital dye image records, contrast can be increased by adjustment of the electronic signal information. When the elements of the

invention are scanned using a reflected beam, the beam travels through the layer units twice. This effectively doubles gamma ( $AD + \Delta \log E$ ) by doubling changes in density ( $\Delta D$ ). Thus, gamma as low as 1.0 or even 0.6 are contemplated and exposure latitudes of up to about 5.0 log E or higher are feasible. Gammas of about less than about 0.55 are preferred. Gammas of between about 0.4 and about 0.5 are especially preferred.

Instead of employing dye-forming couplers, any of the conventional incorporated dye image generating compounds employed in multicolor imaging can be alternatively incorporated in the blue, green and red recording layer units. Dye images can be produced by the selective destruction, formation or physical removal of dyes as a function of exposure. For example, silver dye bleach processes are well known and commercially utilized for forming dye images by the selective destruction of incorporated image dyes. The silver dye bleach process is illustrated by *Research Disclosure*, Item 38957, X. Dye image formers and modifiers, A. Silver dye bleach.

It is also well known that pre-formed image dyes can be incorporated in blue, green and red recording layer units, the dyes being chosen to be initially immobile, but capable of releasing the dye chromophore in a mobile moiety as a function of entering into a redox reaction with oxidized developing agent. These compounds are commonly referred to as redox dye releasers (RDR's). By washing out the released mobile dyes, a retained dye image is created that can be scanned. It is also possible to transfer the released mobile dyes to the photographic processing element of this invention, where they are immobilized in a mordant layer. The image-bearing element can then be scanned. When scanning is conducted with the sheet remaining an integral part of the element, the sheet typically contains a transparent support, the dye image bearing mordant layer just beneath the support, and a white reflective layer just beneath the mordant layer. Where the sheet is peeled from the color negative element to facilitate scanning of the dye image, the support can be reflective, as is commonly the choice when the dye image is intended to be viewed, or transparent, which allows transmission scanning of the dye image. RDR's as well as dye image transfer systems in which they are incorporated are described in *Research Disclosure*, Vol. 151, November 1976, Item 15162.

It is also recognized that the dye image can be provided by compounds that are initially mobile, but are rendered immobile during imagewise development. Image transfer systems utilizing imaging dyes of this type have long been used in previously disclosed dye image transfer systems. These and other image transfer systems compatible with the practice of the invention are disclosed in *Research Disclosure*, Vol. 176, December 1978, Item 17643, XXIII. Image transfer systems.

A number of modifications of color negative elements have been suggested for accommodating scanning, as illustrated by *Research Disclosure*, XIV. Scan facilitating features. These systems to the extent compatible with the color negative element constructions described above are contemplated for use in the practice of this invention.

It is also contemplated that the imaging element for use with this invention may be used with non-conventional sensitization schemes. For example, instead of using imaging layers sensitized to the red, green, and blue regions of the spectrum, the light-sensitive material may have one white-sensitive layer to record scene luminance, and two color-sensitive layers to record scene chrominance. Following development, the resulting image can be scanned and digi-

tally reprocessed to reconstruct the full colors of the original scene as described by Arakawa et al U.S. Pat. No. 5,962,205, the disclosures of which are incorporated herein by reference. The imaging element may also comprise a pan-sensitized emulsion with accompanying color-separation exposure. In this embodiment, the developers of the invention would give rise to a colored or neutral image which, in conjunction with the separation exposure, would enable full recovery of the original scene color values. In such an element, the image may be formed by either developed silver density, a combination of one or more conventional couplers, or "black" couplers such as resorcinol couplers. The separation exposure may be made either sequentially through appropriate filters, or simultaneously through a system of spatially discreet filter elements (commonly called a "color filter array").

The imaging element for use with the invention may also be a black and white image-forming material comprised, for example, of a pan-sensitized silver halide emulsion and a developer of the invention. In this embodiment, the image may be formed by developed silver density following processing, or by a coupler that generates a dye which can be used to carry the neutral image tone scale.

When conventional yellow, magenta, and cyan image dyes are formed to read out the recorded scene exposures following chemical development of conventional exposed color photographic materials, the response of the red, green, and blue color recording units of the element can be accurately discerned by examining their densities. Densitometry is the measurement of transmitted light by a sample using selected colored filters to separate the imagewise response of the RGB image dye forming units into relatively independent channels. It is common to use Status M filters to gauge the response of color negative film elements intended for optical printing, and Status A filters for color reversal films intended for direct transmission viewing. In integral densitometry, the unwanted side and tail absorptions of the imperfect image dyes leads to a small amount of channel mixing, where part of the total response of, for example, a magenta channel may come from off-peak absorptions of either the yellow or cyan image dyes records, or both, in neutral characteristic curves. Such artifacts may be negligible in the measurement of a film's spectral sensitivity. By appropriate mathematical treatment of the integral density response, these unwanted off-peak density contributions can be completely corrected providing analytical densities, where the response of a given color record is independent of the spectral contributions of the other image dyes. Analytical density determination has been summarized in the *SPSE Handbook of Photographic Science and Engineering*, W. Thomas, editor, John Wiley and Sons, New York, 1973, Section 15.3, Color Densitometry, pp. 840-848.

Image noise can be reduced, where the images are obtained by scanning exposed and processed color negative film elements to obtain a manipulatable electronic record of the image pattern, followed by reconversion of the adjusted electronic record to a viewable form. Image sharpness and colorfulness can be increased by designing layer gamma ratios to be within a narrow range while avoiding or minimizing other performance deficiencies, where the color record is placed in an electronic form prior to recreating a color image to be viewed.

The term "gamma ratio" when applied to a color recording layer unit refers to the ratio determined by dividing the color gamma of a cited layer unit after imagewise color separation exposure and process that enables development of primarily that layer unit by the color gamma of the same

layer unit after imagewise white light exposure and process that enables development of all layer units. This term relates to the degree of color saturation available from that layer unit after conventional optical printing. Larger values of the gamma ratio indicate enhanced degrees of color saturation under optical printing conditions.

Whereas it is impossible to separate image noise from the remainder of the image information, either in printing or by manipulating an electronic image record, it is possible by adjusting an electronic image record that exhibits low noise, as is provided by color negative film elements with low gamma ratios, to improve overall curve shape and sharpness characteristics in a manner that is impossible to achieve by known printing techniques. Thus, images can be recreated from electronic image records derived from such color negative elements that are superior to those similarly derived from conventional color negative elements constructed to serve optical printing applications. The excellent imaging characteristics of the described element are obtained when the gamma ratio for each of the red, green and blue color recording units is less than 1.2. In a more preferred embodiment, the red, green, and blue light-sensitive color forming units each exhibit gamma ratios of less than 1.15. In an even more preferred embodiment, the red and blue light-sensitive color forming units each exhibit gamma ratios of less than 1.10. In a most preferred embodiment, the red, green, and blue light-sensitive color forming units each exhibit gamma ratios of less than 1.10. In all cases, it is preferred that the individual color unit(s) exhibit gamma ratios of less than 1.15, more preferred that they exhibit gamma ratios of less than 1.10 and even more preferred that they exhibit gamma ratios of less than 1.05. The gamma ratios of the layer units need not be equal. These low values of the gamma ratio are indicative of low levels of interlayer interaction, also known as interlayer interimage effects, between the layer units and are believed to account for the improved quality of the images after scanning and electronic manipulation. The apparently deleterious image characteristics that result from chemical interactions between the layer units need not be electronically suppressed during the image manipulation activity. The interactions are often difficult if not impossible to suppress properly using known electronic image manipulation schemes.

Elements having excellent light sensitivity are best employed in the practice of this invention. The elements should have a sensitivity of at least about ISO 50, preferably have a sensitivity of at least about ISO 100, and more preferably have a sensitivity of at least about ISO 200. Elements having a sensitivity of up to ISO 3200 or even higher are specifically contemplated. The speed, or sensitivity, of a color negative photographic element is inversely related to the exposure required to enable the attainment of a specified density above fog after processing. Photographic speed for a color negative element with a gamma of about 0.65 in each color record has been specifically defined by the American National Standards Institute (ANSI) as ANSI Standard Number PH 2.27-1981 (ISO (ASA Speed)) and relates specifically the average of exposure levels required to produce a density of 0.15 above the minimum density in each of the green light-sensitive and least sensitive color recording unit of a color film. This definition conforms to the International Standards Organization (ISO) film speed rating. For the purposes of this application, if the color unit gammas differ from 0.65, the ASA or ISO speed is to be calculated by linearly amplifying or deamplifying the gamma vs. log E (exposure) curve to a value of 0.65 before determining the speed in the otherwise defined manner.

The present invention also contemplates the use of photographic elements in what are often referred to as single use cameras (or "film with lens" units). These cameras are sold with film preloaded in them and the entire camera is returned to a processor with the exposed film remaining inside the camera. The one-time-use cameras employed in this invention can be any of those known in the art. These cameras can provide specific features as known in the art such as shutter means, film winding means, film advance means, waterproof housings, single or multiple lenses, lens selection means, variable aperture, focus or focal length lenses, means for monitoring lighting conditions, means for adjusting shutter times or lens characteristics based on lighting conditions or user provided instructions, and means for camera recording use conditions directly on the film. These features include, but are not limited to: providing simplified mechanisms for manually or automatically advancing film and resetting shutters as described at Skarman, U.S. Pat. No. 4,226,517; providing apparatus for automatic exposure control as described at Matterson et al, U.S. Pat. No. 4,345,835; moisture-proofing as described at Fujimura et al, U.S. Pat. No. 4,766,451; providing internal and external film casings as described at Ohmura et al, U.S. Pat. No. 4,751,536; providing means for recording use conditions on the film as described at Taniguchi et al, U.S. Pat. No. 4,780,735; providing lens fitted cameras as described at Arai, U.S. Pat. No. 4,804,987; providing film supports with superior anti-curl properties as described at Sasaki et al, U.S. Pat. No. 4,827,298; providing a viewfinder as described at Ohmura et al, U.S. Pat. No. 4,812,863; providing a lens of defined focal length and lens speed as described at Ushiro et al, U.S. Pat. No. 4,812,866; providing multiple film containers as described at Nakayama et al, U.S. Pat. No. 4,831,398 and at Ohmura et al, U.S. Pat. No. 4,833,495; providing films with improved anti-friction characteristics as described at Shiba, U.S. Pat. No. 4,866,469; providing winding mechanisms, rotating spools, or resilient sleeves as described at Mochida, U.S. Pat. No. 4,884,087; providing a film patron or cartridge removable in an axial direction as described by Takei et al at U.S. Pat. No. 4,890,130 and 5,063,400; providing an electronic flash means as described at Ohmura et al, U.S. Pat. No. 4,896,178; providing an externally operable member for effecting exposure as described at Mochida et al, U.S. Pat. No. 4,954,857; providing film support with modified sprocket holes and means for advancing said film as described at Murakami, U.S. Pat. No. 5,049,908; providing internal mirrors as described at Hara, U.S. Pat. No. 5,084,719; and providing silver halide emulsions suitable for use on tightly wound spools as described at Yagi et al, European Patent Application 0,466,417 A.

While the film may be mounted in the one-time-use camera in any manner known in the art, it is especially preferred to mount the film in the one-time-use camera such that it is taken up on exposure by a thrust cartridge. Thrust cartridges are disclosed by Kataoka et al U.S. Pat. No. 5,226,613; by Zander U.S. Pat. No. 5,200,777; by Dowling et al U.S. Pat. No. 5,031,852; and by Robertson et al U.S. Pat. No. 4,834,306. Narrow bodied one-time-use cameras suitable for employing thrust cartridges in this way are described by Tobioka et al U.S. Pat. No. 5,692,221. More generally, the size limited cameras most useful as one-time-use cameras will be generally rectangular in shape and can meet the requirements of easy handling and transportability in, for example, a pocket, when the camera as described herein has a limited volume. The camera should have a total volume of less than about 450 cubic centimeters (cc's), preferably less than 380 cc, more preferably less than 300 cc,

and most preferably less than 220 cc. The depth-to-height-to-length proportions of such a camera will generally be in an about 1:2:4 ratio, with a range in each of about 25% so as to provide comfortable handling and pocketability. Generally the minimum usable depth is set by the focal length of the incorporated lens and by the dimensions of the incorporated film spools and cartridge. The camera will preferably have the majority of corners and edges finished with a radius-of-curvature of between about 0.2 and 3 centimeters. The use of thrust cartridges allows a particular advantage in this invention by providing easy scanner access to particular scenes photographed on a roll while protecting the film from dust, scratches, and abrasion, all of which tend to degrade the quality of an image.

While any known taking lens may be employed in the cameras of this invention, the taking lens mounted on the single-use cameras of the invention are preferably single aspherical plastic lenses. The lenses will have a focal length between about 10 and 100 mm, and a lens aperture between f/2 and f/32. The focal length is preferably between about 15 and 60 mm and most preferably between about 20 and 40 mm. For pictorial applications, a focal length matching to within 25% the diagonal of the rectangular film exposure area is preferred. Lens apertures of between f/2.8 and f/22 are contemplated with a lens aperture of about f/4 to f/16 being preferred. The lens MTF can be as low as 0.6 or less at a spatial frequency of 20 lines per millimeter (1 pm) at the film plane, although values as high as 0.7 or most preferably 0.8 or more are contemplated. Higher lens MTF values generally allow sharper pictures to be produced. Multiple lens arrangements comprising two, three, or more component lens elements consistent with the functions described above are specifically contemplated.

Cameras may contain a built-in processing capability, for example a heating element. Designs for such cameras including their use in an image capture and display system are disclosed in U.S. patent application Ser. No. 09/388,573, incorporated herein by reference.

Photographic elements of the present invention are preferably imagewise exposed using any of the known techniques, including those described in *Research Disclosure I*, section XVI. This typically involves exposure to light in the visible region of the spectrum, and typically such exposure is of a live image through a lens, although exposure can also be exposure to a stored image (such as a computer stored image) by means of light emitting devices (such as light emitting diodes, CRT and the like). Exposures are monochromatic, orthochromatic, or panchromatic depending upon the spectral sensitization of the photographic silver halide.

The elements as discussed above may serve as origination material for some or all of the following processes: image scanning to produce an electronic rendition of the capture image, and subsequent digital processing of that rendition to manipulate, store, transmit, output, or display electronically that image.

The sheet containing an ion exchanged reducing agent of this invention may be used during the processing of photographic elements that contain any or all of the features discussed, but are intended for different forms of processing. These types of systems will be described in detail below.

Type I: Thermal process systems (photothermographic), where processing is initiated solely by the application of heat to the imaging element.

Type II: Low volume systems, where film processing is initiated by contact to a processing solution, but where the processing solution volume is comparable to the total

volume of the imaging layer to be processed. This type of system may include the addition of non solution processing aids, such as the application of heat or of a laminate layer that is applied at the time of processing.

Type III: Conventional photographic systems, where film elements are processed by contact with conventional photographic processing solutions, and the volume of such solutions is very large in comparison to the volume of the imaging layer.

Type I: Photothermographic Systems

The sheet containing ion-exchanged reducing agent may be used to provide developer to a photothermographic element. Photothermographic elements of the type described in Research Disclosure 17029 (Research Disclosure I) are included by reference. The photothermographic elements may be of type A or type B as disclosed in Research Disclosure I. Type A elements contain in reactive association a photosensitive silver halide, a reducing agent or developer, an activator, and a coating vehicle or binder. In these systems development occurs by reduction of silver ions in the photosensitive silver halide to metallic silver. Type B systems can contain all of the elements of a type A system in addition to a salt or complex of an organic compound with silver ion. In these systems, this organic complex is reduced during development to yield silver metal. The organic silver salt will be referred to as the silver donor. References describing such imaging elements include, for example, U.S. Pat. Nos. 3,457,075; 4,459,350; 4,264,725 and 4,741,992.

The photothermographic element comprises a photosensitive component that consists essentially of photographic silver halide. In the type B photothermographic material it is believed that the latent image silver from the silver halide acts as a catalyst for the described image-forming combination upon processing. In these systems, a preferred concentration of photographic silver halide is within the range of 0.01 to 100 moles of photographic silver halide per mole of silver donor in the photothermographic material.

The Type B photothermographic element comprises an oxidation-reduction image forming combination that contains an organic silver salt oxidizing agent. The organic silver salt is a silver salt which is comparatively stable to light, but aids in the formation of a silver image when heated to 80° C. or higher in the presence of an exposed photocatalyst (i.e., the photosensitive silver halide) and a reducing agent.

Suitable organic silver salts include silver salts of organic compounds having a carboxyl group. Preferred examples thereof include a silver salt of an aliphatic carboxylic acid and a silver salt of an aromatic carboxylic acid. Preferred examples of the silver salts of aliphatic carboxylic acids include silver behenate, silver stearate, silver oleate, silver laurate, silver caprate, silver myristate, silver palmitate, silver maleate, silver fumarate, silver tartarate, silver furoate, silver linoleate, silver butyrate and silver camphorate, mixtures thereof, etc. Silver salts which are substitutable with a halogen atom or a hydroxyl group can also be effectively used. Preferred examples of the silver salts of aromatic carboxylic acid and other carboxyl group-containing compounds include silver benzoate, a silver-substituted benzoate such as silver 3,5-dihydroxybenzoate, silver o-methylbenzoate, silver m-methylbenzoate, silver p-methylbenzoate, silver 2,4-dichlorobenzoate, silver acetamidobenzoate, silver p-phenylbenzoate, etc., silver gallate, silver tannate, silver phthalate, silver terephthalate, silver salicylate, silver phenylacetate, silver pyromellitate, a silver salt of 3-carboxymethyl-4-methyl-4-thiazoline-2-thione or the like as described in U.S. Pat. No. 3,785,830,

and silver salt of an aliphatic carboxylic acid containing a thioether group as described in U.S. Pat. No. 3,330,663.

Silver salts of mercapto or thione substituted compounds having a heterocyclic nucleus containing 5 or 6 ring atoms, at least one of which is nitrogen, with other ring atoms including carbon and up to two hetero-atoms selected from among oxygen, sulfur and nitrogen are specifically contemplated. Typical preferred heterocyclic nuclei include triazole, oxazole, thiazole, thiazoline, imidazoline, 10 imidazole, diazole, pyridine and triazine. Preferred examples of these heterocyclic compounds include a silver salt of 3-mercaptop-4-phenyl-1,2,4 triazole, a silver salt of 2-mercaptopbenzimidazole, a silver salt of 2-mercaptop-5-aminothiadiazole, a silver salt of 2-(2-ethyl-glycolamido) 15 benzothiazole, a silver salt of 5-carboxylic-1-methyl-2-phenyl-4-thiopyridine, a silver salt of mercaptotriazine, a silver salt of 2-mercaptopbenzoxazole, a silver salt as described in U.S. Pat. No. 4,123,274, for example, a silver salt of 1,2,4-mercaptopthiazole derivative such as a silver salt 20 of 3-amino-5-benzylthio-1,2,4-thiazole, a silver salt of a thione compound such as a silver salt of 3-(2-carboxyethyl)-4-methyl-4-thiazoline-2-thione as disclosed in U.S. Pat. No. 3,201,678. Examples of other useful mercapto or thione substituted compounds that do not contain a heterocyclic 25 nucleus are illustrated by the following: a silver salt of thioglycolic acid such as a silver salt of a S-alkylthioglycolic acid (wherein the alkyl group has from 12 to 22 carbon atoms) as described in Japanese patent application 28221/73, a silver salt of a dithiocarboxylic acid such as a silver salt 30 of dithioacetic acid, and a silver salt of thioamide.

Furthermore, a silver salt of a compound containing an imino group can be used. Preferred examples of these compounds include a silver salt of benzotriazole and a derivative thereof as described in Japanese patent publications 30270/69 and 18146/70, for example a silver salt of benzotriazole or methylbenzotriazole, etc., a silver salt of a halogen substituted benzotriazole, such as a silver salt of 5-chlorobenzotriazole, etc., a silver salt of 1,2,4-triazole, a silver salt of 3-amino-5-mercaptopbenzyl-1,2,4-triazole, of 40 1H-tetrazole as described in U.S. Pat. No. 4,220,709, a silver salt of imidazole and an imidazole derivative, and the like.

It is also found convenient to use silver half soap, of which an equimolar blend of a silver behenate with behenic acid, prepared by precipitation from aqueous solution of the 45 sodium salt of commercial behenic acid and analyzing about 14.5 percent silver, represents a preferred example. Transparent sheet materials made on transparent film backing require a transparent coating and for this purpose the silver behenate full soap, containing not more than about 4 or 5 percent of free behenic acid and analyzing about 25.2 percent silver may be used. A method for making silver soap dispersions is well known in the art and is disclosed in Research Disclosure October 1983 (23419) and U.S. Pat. No. 3,985,565.

Silver salts complexes may also be prepared by mixture of aqueous solutions of a silver ionic species, such as silver nitrate, and a solution of the organic ligand to be complexed with silver. The mixture process may take any convenient form, including those employed in the process of silver 50 halide precipitation. A stabilizer may be used to avoid flocculation of the silver complex particles. The stabilizer may be any of those materials known to be useful in the photographic art, such as, but not limited to, gelatin, polyvinyl alcohol or polymeric or monomeric surfactants.

The photosensitive silver halide grains and the organic silver salt are coated so that they are in catalytic proximity during development. They can be coated in contiguous

layers, but are preferably mixed prior to coating. Conventional mixing techniques are illustrated by Research Disclosure, Item 17029, cited above, as well as U.S. Pat. No. 3,700,458 and published Japanese patent applications Nos. 32928/75, 13224/74, 17216/75 and 42729/76.

A reducing agent in addition to that provided during processing by the sheet comprising an ion exchanges reducing agent may be included. The reducing agent for the organic silver salt may be any material, preferably organic material, that can reduce silver ion to metallic silver. Conventional photographic developers such as 3-pyrazolidinones, hydroquinones, p-aminophenols, p-phenylenediamines and catechol are useful, but hindered phenol reducing agents are preferred. The reducing agent is preferably present in a concentration ranging from 5 to 25 percent of the photothermographic layer.

A wide range of reducing agents has been disclosed in dry silver systems including amidoximes such as phenylamidoxime, 2-thienylamidoxime and p-phenoxyphenylamidoxime, azines (e.g., 4-hydroxy-3,5-dimethoxybenzaldehydeazine); a combination of aliphatic carboxylic acid aryl hydrazides and ascorbic acid, such as 2,2'-bis(hydroxymethyl)propionylbetaphenyl hydrazide in combination with ascorbic acid; an combination of polyhydroxybenzene and hydroxylamine, a reductone and/or a hydrazine, e.g., a combination of hydroquinone and bis(ethoxyethyl)hydroxylamine, piperidinohexose reductone or formyl-4-methylphenylhydrazine, hydroxamic acids such as phenylhydroxamic acid, p-hydroxyphenyl-hydroxamic acid, and o-alaninehydroxamic acid; a combination of azines and sulfonamidophenols, e.g., phenothiazine and 2,6-dichloro-4-benzenesulfonamidophenol;  $\alpha$ -cyanophenylacetic acid derivatives such as ethyl  $\alpha$ -cyano-2-methylphenylacetate, ethyl  $\alpha$ -cyano-phenylacetate; bis- $\beta$ -naphthols as illustrated by 2,2'-dihydroxy-1,1'-binaphthyl, 6,6'-dibromo-2,2'-dihydroxy-1,1'-binaphthyl, and bis(2-hydroxy-1-naphthyl) methane; a combination of bis- $\beta$ -naphthol and a 1,3-dihydroxybenzene derivative, (e. g., 2,4-dihydroxybenzophenone or 2,4-dihydroxyacetophenone); 5-pyrazolones such as 3-methyl-1-phenyl-5-pyrazolone; reductones as illustrated by dimethylaminohexose reductone, anhydrodihydroaminohexose reductone, and anhydroadihydro-piperidone-hexose reductone; sulfamidophenol reducing agents such as 2,6-dichloro-4-benzene-sulfon-amido-phenol, and p-benzenesulfonamidophenol; 2-phenylindane-1,3-dione and the like; chromans such as 2,2-dimethyl-7-t-butyl-6-hydroxychroman; 1,4-dihydropyridines such as 2,6-dimethoxy-3,5-dicarbethoxy-1,4-dihydropyridene; bisphenols, e.g., bis(2-hydroxy-3-t-butyl-5-methylphenyl)-methane; 2,2-bis(4-hydroxy-3-methylphenyl)-propane; 4,4-ethylidene-bis(2-t-butyl-6-methylphenol); and 2,2-bis(3,5-dimethyl-4-hydroxyphenyl)propane; ascorbic acid derivatives, e.g., 1-ascorbyl-palmitate, ascorbylsteareate and unsaturated aldehydes and ketones, such as benzyl and diacetyl; pyrazolidin-3-ones; and certain indane-1,3-diones.

An optimum concentration of organic reducing agent in the photothermographic element varies depending upon such factors as the particular photothermographic element, desired image, processing conditions, the particular organic silver salt and the particular oxidizing agent.

The photothermographic element can comprise a toning agent, also known as an activator-toner or toner-accelerator. Combinations of toning agents are also useful in the photothermographic element. Examples of useful toning agents and toning agent combinations are described in, for example, *Research Disclosure*, June 1978, Item No. 17029

and U.S. Pat. No. 4,123,282. Examples of useful toning agents include, for example, phthalimide, N-hydroxyphthalimide, N-potassium-phthalimide, succinimide, N-hydroxy-1,8-naphthalimide, phthalazine, 1-(2H)-phthalazinone, 2-acetylphthalazinone, salicylanilide, benzamide, and dimethylurea. These agents may also optionally be supplied by the photographic processing sheet of the invention.

Post-processing image stabilizers and latent image keeping stabilizers are useful in the photothermographic element. Any of the stabilizers known in the photothermographic art are useful for the described photothermographic element. Illustrative examples of useful stabilizers include photolytically active stabilizers and stabilizer precursors as described in, for example, U.S. Pat. No. 4,459,350. Other examples of useful stabilizers include azole thioethers and blocked azolinethione stabilizer precursors and carbamoyl stabilizer precursors, such as described in U.S. Pat. No. 3,877,940. These agents may also optionally be supplied by the photographic processing sheet of the invention.

The photothermographic elements preferably contain various colloids and polymers alone or in combination as vehicles and binders and in various layers. Useful materials are hydrophilic or hydrophobic. They are transparent or translucent and include both naturally occurring substances, such as gelatin, gelatin derivatives, cellulose derivatives, polysaccharides, such as dextran, gum arabic and the like; and synthetic polymeric substances, such as water-soluble polyvinyl compounds like poly(vinylpyrrolidone) and acrylamide polymers. Other synthetic polymeric compounds that are useful include dispersed vinyl compounds such as in latex form and particularly those that increase dimensional stability of photographic elements. Effective polymers include water insoluble polymers of acrylates, such as alkylacrylates and methacrylates, acrylic acid, sulfoacrylates, and those that have cross-linking sites. Preferred high molecular weight materials and resins include poly(vinyl butyral), cellulose acetate butyrate, poly(methylmethacrylate), poly(vinylpyrrolidone), ethyl cellulose, polystyrene, poly(vinylchloride), chlorinated rubbers, polyisobutylene, butadiene-styrene copolymers, copolymers of vinyl chloride and vinyl acetate, copolymers of vinylidene chloride and vinyl acetate, poly(vinyl alcohol) and polycarbonates. When coatings are made using organic solvents, organic soluble resins may be coated by direct mixture into the coating formulations. When coating from aqueous solution, any useful organic soluble materials may be incorporated as a latex or other fine particle dispersion.

Photothermographic elements as described can contain addenda that are known to aid in formation of a useful image. The photothermographic element can contain development modifiers that function as speed increasing compounds, sensitizing dyes, hardeners, antistatic agents, plasticizers and lubricants, coating aids, brighteners, absorbing and filter dyes, such as described in *Research Disclosure*, December 1978, Item No. 17643 and *Research Disclosure*, June 1978, Item No. 17029. These agents may also optionally be supplied by the photographic processing sheet of the invention.

The layers of the photothermographic element are coated on a support by coating procedures known in the photographic art, including dip coating, air knife coating, curtain coating or extrusion coating using hoppers. If desired, two or more layers are coated simultaneously.

A photothermographic element as described preferably comprises a thermal stabilizer to help stabilize the photothermographic element prior to exposure and processing.

Such a thermal stabilizer provides improved stability of the photothermographic element during storage. Preferred thermal stabilizers are 2-bromo-2-arylsulfonylacetamides, such as 2-bromo-2-p-tolylsulfonylacetamide; 2-(tribromomethyl sulfonyl)benzothiazole; and 6-substituted-2,4-bis (tribromomethyl)-s-triazines, such as 6-methyl or 6-phenyl-2,4-bis(tribromomethyl)-s-triazine. Imagewise exposure is preferably for a time and intensity sufficient to produce a developable latent image in the photothermographic element.

After imagewise exposure of the photothermographic element, the resulting latent image can be developed in a variety of ways. The simplest is by overall heating the element in contact with the photographic processing sheet of this invention to thermal processing temperature. This overall heating merely involves heating the photothermographic element to a temperature within the range of about 90° C. to about 180° C. until a developed image is formed, such as within about 0.5 to about 60 seconds. By increasing or decreasing the thermal processing temperature a shorter or longer time of processing is useful. A preferred thermal processing temperature is within the range of about 100° C. to about 160° C. Heating means known in the photothermographic arts are useful for providing the desired processing temperature for the exposed photothermographic element. The heating means is, for example, a simple hot plate, iron, roller, heated drum, microwave heating means, heated air, vapor or the like.

It is contemplated that the design of the processor for the photothermographic element be linked to the design of the cassette or cartridge used for storage and use of the element. Further, data stored on the film or cartridge may be used to modify processing conditions or scanning of the element. Methods for accomplishing these steps in the imaging system are disclosed in commonly assigned, co-pending U.S. patent applications Ser. Nos. 09/206586, 09/206,612, and 09/206,583 filed Dec. 7, 1998, which are incorporated herein by reference. The use of an apparatus whereby the processor can be used to write information onto the element, information which can be used to adjust processing, scanning, and image display is also envisaged. This system is disclosed in U.S. patent applications Ser. Nos. 09/206,914 filed Dec. 7, 1998 and 09/333,092 filed Jun. 15, 1999, which are incorporated herein by reference.

Thermal processing is preferably carried out under ambient conditions of pressure and humidity. Conditions outside of normal atmospheric pressure and humidity are useful.

The components of the photothermographic element can be in any location in the element that provides the desired image. If desired, one or more of the components can be in one or more layers of the element. For example, in some cases, it is desirable to include certain percentages of the reducing agent, toner, stabilizer and/or other addenda in the overcoat layer over the photothermographic image recording layer of the element. This, in some cases, reduces migration of certain addenda in the layers of the element.

#### Type II: Low Volume Processing

In accordance with another aspect of this invention the sheet containing ion exchanged reducing agent is used during the processing of a photographic element intended for low volume processing. Low volume processing is defined as processing where the volume of applied solution is between about 0.1 to about 10 times, preferably about 0.5 to about 10 times, the volume of solution required to swell the photographic element. This processing may take place by a combination of solution application, external layer lamination, and heating. The low volume processing system

may contain any of the elements described above for Type I: Photothermographic systems. In addition, it is specifically contemplated that any components described in the preceding sections that are not necessary for the formation or stability of latent image in the origination film element can be removed from the film element altogether and contacted at any time after exposure for the purpose of carrying out photographic processing, using the methods described below.

10 The Type II photographic element may receive some or all of the following treatments:

(I) Application of a solution directly to the film by any means, including spray, inkjet, coating, gravure process and the like.

15 (II) Soaking of the film in a reservoir containing a processing solution. This process may also take the form of dipping or passing an element through a small cartridge.

(III) Lamination of an auxiliary processing element to the imaging element. The laminate may have the purpose of providing processing chemistry, removing spent chemistry, or transferring image information from the latent image recording film element. The transferred image may result from a dye, dye precursor, or silver containing compound being transferred in a image-wise manner to the auxiliary processing element. The auxiliary processing element, for example, may be the photographic processing sheet of this invention.

(IV) Heating of the element by any convenient means, including a simple hot plate, iron, roller, heated drum, microwave heating means, heated air, vapor, or the like. Heating may be accomplished before, during, after, or throughout any of the preceding treatments I-III. Heating may cause processing temperatures ranging from room temperature to 100° C.

#### 35 Type III: Conventional Systems

In accordance with another aspect of this invention the sheet containing ion exchanged reducing agent is used during the processing of a conventional photographic element.

40 Conventional photographic elements in accordance with the invention can be processed in any of a number of well-known photographic processes utilizing any of a number of well-known conventional photographic processing solutions, described, for example, in *Research Disclosure I*, or in T. H. James, editor, *The Theory of the Photographic Process*, 4th Edition, Macmillan, N.Y., 1977. The development process may take place for any length of time and any process temperature that is suitable to render an acceptable image. In these cases the presence of ion exchanged develop-

45 ers of the invention may be used to provide development in one or more color records of the element, supplementary to the development provided by the developer in the processing solution to give improved signal in a shorter time of development or with lowered laydowns of imaging materials, or to give balanced development in all color records. In the case of processing a negative working element, the element is treated with a color developer (that is one which will form the colored image dyes with the color couplers), and then with a oxidizer and a solvent to remove silver and silver halide. In the case of processing a reversal color element, the element is first treated with a black and white developer (that is, a developer which does not form colored dyes with the coupler compounds) followed by a treatment to fog silver halide (usually chemical fogging or light fogging), followed by treatment with a color developer. Preferred color developing agents are p-phenylenediamines.

50 Especially preferred are:

55

60

65

4-amino N,N-diethylaniline hydrochloride,  
 4-amino-3-methyl-N,N-diethylaniline hydrochloride,  
 4-amino-3-methyl-N-ethyl-N-(2-(methanesulfonamido)ethylaniline sesquisulfate hydrate,  
 4-amino-3-methyl-N-ethyl-N-(2-hydroxyethyl)aniline sulfate,  
 4-amino-3- $\alpha$ -(methanesulfonamido)ethyl-N,N-diethylaniline hydrochloride and  
 4-amino-N-ethyl-N-(2-methoxyethyl)-m-toluidine di-p-toluene sulfonic acid.

Dye images can be formed or amplified by processes which employ in combination with a dye-image-generating reducing agent an inert transition metal-ion complex oxidizing agent, as illustrated by Bissonette U.S. Pat. Nos. 3,748,138, 3,826,652, 3,862,842 and 3,989,526 and Travis U.S. Pat. No. 3,765,891, and/or a peroxide oxidizing agent as illustrated by Matejec U.S. Pat. No. 3,674,490, Research Disclosure, Vol. 116, December, 1973, Item 11660, and Bissonette Research Disclosure, Vol. 148, August, 1976, Items 14836, 14846 and 14847. The photographic elements can be particularly adapted to form dye images by such processes as illustrated by Dunn et al U.S. Pat. No. 3,822,129, Bissonette U.S. Pat. Nos. 3,834,907 and 3,902,905, Bissonette et al U.S. Pat. No. 3,847,619, Mowrey U.S. Pat. No. 3,904,413, Hirai et al U.S. Pat. No. 4,880,725, Iwano U.S. Pat. No. 4,954,425, Marsden et al U.S. Pat. No. 4,983,504, Evans et al U.S. Pat. No. 5,246,822, Twist U.S. Pat. No. 5,324,624, Fyson EPO 0 487 616, Tannahill et al WO 90/13059, Marsden et al WO 90/13061, Grimsey et al WO 91/16666, Fyson WO 91/17479, Marsden et al WO 92/01972, Tannahill WO 92/05471, Henson WO 92/07299, Twist WO 93/01524 and WO 93/11460 and Wingender et al German OLS 4,211,460.

Development may be followed by bleach-fixing, to remove silver or silver halide, washing and drying.

In embodiments of the invention in which an ion exchanged developer is used in a processing sheet, it is contemplated that the processing solution will contain little, if any, developer. However, in certain embodiments of the invention it may be useful to provide a developer in the processing solution in addition to that provided by the processing sheet.

Once yellow, magenta, and cyan dye image records have been formed in the processed photographic elements of the invention, conventional techniques can be employed for retrieving the image information for each color record and manipulating the record for subsequent creation of a color balanced viewable image. For example, it is possible to scan the photographic element successively within the blue, green, and red regions of the spectrum or to incorporate blue, green, and red light within a single scanning beam that is divided and passed through blue, green, and red filters to form separate scanning beams for each color record. A simple technique is to scan the photographic element point-by-point along a series of laterally offset parallel scan paths. The intensity of light passing through the element at a scanning point is noted by a sensor which converts radiation received into an electrical signal. Most generally this electronic signal is further manipulated to form a useful electronic record of the image. For example, the electrical signal can be passed through an analog-to-digital converter and sent to a digital computer together with location information required for pixel (point) location within the image. In another embodiment, this electronic signal is encoded with colorimetric or tonal information to form an electronic record that is suitable to allow reconstruction of the image into viewable forms such as computer monitor displayed images, television images, printed images, and so forth.

It is contemplated that many of imaging elements of this invention will be scanned prior to the removal of silver halide from the element. The remaining silver halide yields a turbid coating, and it is found that improved scanned image quality for such a system can be obtained by the use of scanners that employ diffuse illumination optics. Any technique known in the art for producing diffuse illumination can be used. Preferred systems include reflective systems, that employ a diffusing cavity whose interior walls are specifically designed to produce a high degree of diffuse reflection, and transmissive systems, where diffusion of a beam of specular light is accomplished by the use of an optical element placed in the beam that serves to scatter light. Such elements can be either glass or plastic that either incorporate a component that produces the desired scattering, or have been given a surface treatment to promote the desired scattering.

One of the challenges encountered in producing images from information extracted by scanning is that the number of pixels of information available for viewing is only a fraction of that available from a comparable classical photographic print. It is, therefore, even more important in scan imaging to maximize the quality of the image information available. Enhancing image sharpness and minimizing the impact of aberrant pixel signals (i.e., noise) are common approaches to enhancing image quality. A conventional technique for minimizing the impact of aberrant pixel signals is to adjust each pixel density reading to a weighted average value by factoring in readings from adjacent pixels, closer adjacent pixels being weighted more heavily.

The elements for use with the invention can have density calibration patches derived from one or more patch areas on a portion of unexposed photographic recording material that was subjected to reference exposures, as described by Wheeler et al U.S. Pat. No. 5,649,260, Koeng et al U.S. Pat. No. 5,563,717, and by Cosgrove et al U.S. Pat. No. 5,644,647.

Illustrative systems of scan signal manipulation, including techniques for maximizing the quality of image records, are disclosed by Bayer U.S. Pat. No. 4,553,156; Urabe et al U.S. Pat. No. 4,591,923; Sasaki et al U.S. Pat. No. 4,631,578; Alkofer U.S. Pat. No. 4,654,722; Yamada et al U.S. Pat. No. 4,670,793; Klees U.S. Pat. Nos. 4,694,342 and 4,962,542; Powell U.S. Pat. No. 4,805,031; Mayne et al U.S. Pat. No. 4,829,370; Abdulwahab U.S. Pat. No. 4,839,721; Matsunawa et al U.S. Pat. Nos. 4,841,361 and 4,937,662; Mizukoshi et al U.S. Pat. No. 4,891,713; Petilli U.S. Pat. No. 4,912,569; Sullivan et al U.S. Pat. Nos. 4,920,501 and 5,070,413; Kimoto et al U.S. Pat. No. 4,929,979; Hirosawa et al U.S. Pat. No. 4,972,256; Kaplan U.S. Pat. No. 4,977,521; Sakai U.S. Pat. No. 4,979,027; Ng U.S. Pat. No. 5,003,494; Katayama et al U.S. Pat. No. 5,008,950; Kimura et al U.S. Pat. No. 5,065,255; Osamu et al U.S. Pat. No. 5,051,842; Lee et al U.S. Pat. No. 5,012,333; Bowers et al U.S. Pat. No. 5,107,346; Telle U.S. Pat. No. 5,105,266; MacDonald et al U.S. Pat. No. 5,105,469; and Kwon et al U.S. Pat. No. 5,081,692. Techniques for color balance adjustments during scanning are disclosed by Moore et al U.S. Pat. No. 5,049,984 and Davis U.S. Pat. No. 5,541,645.

The digital color records once acquired are in most instances adjusted to produce a pleasingly color balanced image for viewing and to preserve the color fidelity of the image bearing signals through various transformations or renderings for outputting, either on a video monitor or when printed as a conventional color print. Preferred techniques for transforming image bearing signals after scanning are disclosed by Giorgianni et al U.S. Pat. No. 5,267,030, the

disclosures of which are herein incorporated by reference. Further illustrations of the capability of those skilled in the art to manage color digital image information are provided by Giorgianni and Madden *Digital Color Management*, Addison-Wesley, 1998.

FIG. 1 shows, in block diagram form, the manner in which the image information provided by the color negative elements for use with the invention is contemplated to be used. An image scanner 2 is used to scan by transmission an imagewise exposed and photographically processed color negative element 1. The scanning beam is most conveniently a beam of white light that is split after passage through the layer units and passed through filters to create separate image records-red recording layer unit image record (R), green recording layer unit image record (G), and blue recording layer unit image record (B). Instead of splitting the beam, blue, green, and red filters can be sequentially caused to intersect the beam at each pixel location. In still another scanning variation, separate blue, green, and red light beams, as produced by a collection of light emitting diodes, can be directed at each pixel location. As the element 1 is scanned pixel-by-pixel using an array detector, such as an array charge-coupled device (CCD), or line-by-line using a linear array detector, such as a linear array CCD, a sequence of R, G, and B picture element signals are generated that can be correlated with spatial location information provided from the scanner. Signal intensity and location information is fed to a workstation 4, and the information is transformed into an electronic form R', G', and B', which can be stored in any convenient storage device 5.

In motion imaging industries, a common approach is to transfer the color negative film information into a video signal using a telecine transfer device. Two types of telecine transfer devices are most common: (1) a flying spot scanner using photomultiplier tube detectors or (2) CCD's as sensors. These devices transform the scanning beam that has passed through the color negative film at each pixel location into a voltage. The signal processing then inverts the electrical signal in order to render a positive image. The signal is then amplified and modulated and fed into a cathode ray tube monitor to display the image or recorded onto magnetic tape for storage. Although both analog and digital image signal manipulations are contemplated, it is preferred to place the signal in a digital form for manipulation, since the overwhelming majority of computers are now digital and this facilitates use with common computer peripherals, such as magnetic tape, a magnetic disk, or an optical disk.

A video monitor 6, which receives the digital image information modified for its requirements, indicated by R", G", and B", allows viewing of the image information received by the workstation. Instead of relying on a cathode ray tube of a video monitor, a liquid crystal display panel or any other convenient electronic image viewing device can be substituted. The video monitor typically relies upon a picture control apparatus 3, which can include a keyboard and cursor, enabling the workstation operator to provide image manipulation commands for modifying the video image displayed and any image to be recreated from the digital image information.

Any modifications of the image can be viewed as they are being introduced on the video display 6 and stored in the storage device 5. The modified image information R", G", and B" can be sent to an output device 7 to produce a recreated image for viewing. The output device can be any convenient element writer, such as a thermal dye transfer, ink-jet, electrostatic, electrophotographic, or other type of printer suitable for rendering a viewable image. The output

device can be used to control the exposure of a silver halide color paper. The silver halide output medium and/or its method of processing may be conventional or modified according to the present invention. It is the image in the output medium that is ultimately viewed and judged by the end user for noise (granularity), sharpness, contrast, and color balance. The image on a video display may also ultimately be viewed and judged by the end user for noise, sharpness, tone scale, color balance, and color reproduction, as in the case of images transmitted between parties on the World Wide Web of the Internet computer network.

Using an arrangement of the type shown in FIG. 1, the images contained in color negative elements are converted to digital form, manipulated, and recreated in a viewable form following the procedure described in Giorgianni et al U.S. Pat. No. 5,267,030. Color negative recording materials can be used with any of the suitable methods described in U.S. Pat. No. 5,257,030. In one preferred embodiment, Giorgianni et al provides for a method and means to convert the R, G, and B image-bearing signals from a transmission scanner to an image manipulation and/or storage metric which corresponds to the trichromatic signals of a reference image-producing device such as a film or paper writer, thermal printer, video display, etc. The metric values correspond to those which would be required to appropriately 15 reproduce the color image on that device. For example, if the reference image producing device was chosen to be a specific video display, and the intermediary image data metric was chosen to be the R', G', and B' intensity modulating signals (code values) for that reference video display, 20 then for an input film, the R, G, and B image-bearing signals which corresponds to those which would be required to appropriately reproduce the input image on the reference video display. A data-set is generated from which the mathematical 25 transformations to convert R, G, and B image-bearing signals to the aforementioned code values are derived. Exposure patterns, chosen to adequately sample and cover the useful exposure range of the film being calibrated, are created by exposing a pattern generator and are fed to an exposing apparatus. The exposing apparatus produces trichromatic exposures on film to create test images consisting of approximately 150 color patches. Test images may be created using a variety of methods appropriate for the application. These methods include: using exposing apparatus such as a sensitometer, using the output device of a color imaging apparatus, recording images of test objects of known reflectances illuminated by known light sources, or calculating trichromatic exposure values using methods known in the photographic art. If input films of different 30 speeds are used, the overall red, green, and blue exposures must be properly adjusted for each film in order to compensate for the relative speed differences among the films. Each film thus receives equivalent exposures, appropriate for its red, green, and blue speeds. The exposed film is processed 35 chemically. Film color patches are read by transmission scanner which produces R, G, and B image-bearing signals corresponding each color patch. Signal-value patterns of code value pattern generator produces RGB intensity-modulating signals which are fed to the reference video 40 display. The R', G', and B' code values for each test color are adjusted such that a color matching apparatus, which may correspond to an instrument or a human observer, indicates that the video display test colors match the positive film test colors or the colors of a printed negative. A transform apparatus creates a transform relating the R, G, and B image-bearing signal values for the film's test colors to the R', G', and B' code values of the corresponding test colors.

The mathematical operations required to transform R, G, and B image-bearing signals to the intermediary data may consist of a sequence of matrix operations and look-up tables (LUT's).

Referring to FIG. 2, input image-bearing signals R, G, and B are transformed to intermediary data values corresponding to the R', G', and B' output image-bearing signals required to appropriately reproduce the color image on the reference output device as follows:

- (1) The R, G, and B image-bearing signals, which correspond to the measured transmittances of the film, are converted to corresponding densities in the computer used to receive and store the signals from a film scanner by means of 1-dimensional look-up table LUT 1.
- (2) The densities from step (1) are then transformed using matrix 1 derived from a transform apparatus to create intermediary image-bearing signals.
- (3) The densities of step (2) are optionally modified with a 1-dimensional look-up table LUT 2 derived such that the neutral scale densities of the input film are transformed to the neutral scale densities of the reference.
- (4) The densities of step (3) are transformed through a 1-dimensional look-up table LUT 3 to create corresponding R', G', and B' output image-bearing signals for the reference output device.

It will be understood that individual look-up tables are typically provided for each input color. In one embodiment, three 1-dimensional look-up tables can be employed, one for each of a red, green, and blue color record. In another embodiment, a multi-dimensional look-up table can be employed as described by D'Errico at U.S. Pat. No. 4,941,039. It will be appreciated that the output image-bearing signals for the reference output device of step 4 above may be in the form of device-dependent code values or the output image-bearing signals may require further adjustment to become device specific code values. Such adjustment may be accomplished by further matrix transformation or 1-dimensional look-up table transformation, or a combination of such transformations to properly prepare the output image-bearing signals for any of the steps of transmitting, storing, printing, or displaying them using the specified device.

The R, G, and B image-bearing signals from a transmission scanner are converted to an image manipulation and/or storage metric which corresponds to a measurement or description of a single reference image-recording device and/or medium and in which the metric values for all input media correspond to the trichromatic values which would have been formed by the reference device or medium had it captured the original scene under the same conditions under which the input media captured that scene. For example, if the reference image recording medium was chosen to be a specific color negative film, and the intermediary image data metric was chosen to be the measured RGB densities of that reference film, then for an input color negative film according to the invention, the R, G, and B image-bearing signals from a scanner would be transformed to the R', G', and B' density values corresponding to those of an image which would have been formed by the reference color negative film had it been exposed under the same conditions under which the color negative recording material was exposed.

Exposure patterns, chosen to adequately sample and cover the useful exposure range of the film being calibrated, are created by exposing a pattern generator and are fed to an exposing apparatus. The exposing apparatus produces trichromatic exposures on film to create test images consisting of approximately 150 color patches. Test images may

be created using a variety of methods appropriate for the application. These methods include: using exposing apparatus such as a sensitometer, using the output device of a color imaging apparatus, recording images of test objects of known reflectances illuminated by known light sources, or calculating trichromatic exposure values using methods known in the photographic art. If input films of different speeds are used, the overall red, green, and blue exposures must be properly adjusted for each film in order to compensate for the relative speed differences among the films. Each film thus receives equivalent exposures, appropriate for its red, green, and blue speeds. The exposed film is processed chemically. Film color patches are read by a transmission scanner which produces R, G, and B image-bearing signals corresponding each color patch and by a transmission densitometer which produces R', G', and B' density values corresponding to each patch. A transform apparatus creates a transform relating the R, G, and B image-bearing signal values for the film's test colors to the measured R', G', and B' densities of the corresponding test colors of the reference color negative film. In another preferred variation, if the reference image recording medium was chosen to be a specific color negative film, and the intermediary image data metric was chosen to be the predetermined R', G', and B' intermediary densities of step 2 of that reference film, then for an input color negative film according to the invention, the R, G, and B image-bearing signals from a scanner would be transformed to the R', G', and B' intermediary density values corresponding to those of an image which would have been formed by the reference color negative film had it been exposed under the same conditions under which the color negative recording material was exposed.

Thus each input film would yield, insofar as possible, identical intermediary data values corresponding to the R', G', and B' code values required to appropriately reproduce the color image which would have been formed by the reference color negative film on the reference output device. Uncalibrated films may also be used with transformations derived for similar types of films, and the results would be similar to those described.

The mathematical operations required to transform R, G, and B image-bearing signals to the intermediary data metric of this preferred embodiment may consist of a sequence of matrix operations and 1-dimensional LUTs. Three tables are typically provided for the three input colors. It is appreciated that such transformations can also be accomplished in other embodiments by employing a single mathematical operation or a combination of mathematical operations in the computational steps produced by the host computer including, but not limited to, matrix algebra, algebraic expressions dependent on one or more of the image-bearing signals, and n-dimensional LUTs. In one embodiment, matrix 1 of step 2 is a 3x3 matrix. In a more preferred embodiment, matrix 1 of step 2 is a 3x10 matrix. In a preferred embodiment, the 1-dimensional LUT 3 in step 4 transforms the intermediary image-bearing signals according to a color photographic paper characteristic curve, thereby reproducing normal color print image tone scale. In another preferred embodiment, LUT 3 of step 4 transforms the intermediary image-bearing signals according to a modified viewing tone scale that is more pleasing, such as possessing lower image contrast.

Due to the complexity of these transformations, it should be noted that the transformation from R, G, and B to R', G', and B' may often be better accomplished by a 3-dimensional LUT. Such 3-dimensional LUTs may be developed according to the teachings J. D'Errico in U.S. Pat. No. 4,941,039.

It is to be appreciated that while the images are in electronic form, the image processing is not limited to the

specific manipulations described above. While the image is in this form, additional image manipulation may be used including, but not limited to, standard scene balance algorithms (to determine corrections for density and color balance based on the densities of one or more areas within the negative), tone scale manipulations to amplify film under-exposure gamma, non-adaptive or adaptive sharpening via convolution or unsharp masking, red-eye reduction, and non-adaptive or adaptive grain-suppression. Moreover, the image may be artistically manipulated, zoomed, cropped, and combined with additional images or other manipulations known in the art. Once the image has been corrected and any additional image processing and manipulation has occurred, the image may be electronically transmitted to a remote location or locally written to a variety of output devices including, but not limited to, silver halide film or paper writers, thermal printers, electrophotographic printers, ink-jet printers, display monitors, CD disks, optical and magnetic electronic signal storage devices, and other types of storage and display devices as known in the art.

The following examples illustrate the use of ion exchanged reducing agents contained in processing sheets.

#### EXAMPLE 1

##### Preparation of Components for Processing Color Photographic Elements

A series of developer loaded ion exchange particle slurries were prepared. Samples of a commercially available ion exchange resin were loaded with developer as described below. Dispersal of the resulting developer loaded ion exchange particles M1–M7 was accomplished by subjecting the particle slurry samples to a) high shear mixing with a rotor-stator mixer and/or b) repeated collisions with hard, inorganic milling media. Direct synthesis of ion exchange resin particles P1–P3 were accomplished via suspension polymerization.

##### M1

To 40 g of solution A which contained 10 wt. % of DEV-1 and 2.4 wt. % of sodium sulfite were added 10 g of Amberlite™ IR120<sup>+</sup> strongly acidic gel-type ion exchange resin. The mixture was stirred for five minutes, and the resin particles were separated from the liquid phase. The resin particles were washed with distilled, de-ionized water until the pH of a 20% resin slurry was 4.7. The resulting developer loaded resin particles were added to 56.6 g of a solution containing 0.111 g of cetyltrimethylammonium bromide and 0.152 g of sodium sulfite. The resin particle slurry was sheared for 15 minutes with a rotor-stator mixer at ca. 15,000 RPM and milled for 16 hours with 120 cc of 1.8 mm zirconium oxide beads in an 8 oz jar.

##### M2

A sample of Dowex HCR-W2 Na<sup>+</sup> form, spherical beads (strong acid; styrene-DVB copolymer; nuclear sulfonic acid active group; total exchange capacity=3.8 meq/g) was milled with 1 cm zirconium oxide media for 2 weeks and loaded with developer as follows. In 25 ml of water was dissolved 0.48 g of sodium sulfite followed by a 20 minute purge with nitrogen. To the purged solution was added 5.5 g of DEV-1, and 6.3 g of the 80% solids Dowex HCR-W2 milled dispersion. The resultant dispersion was shaken for 4 hours. The final resin was isolated by centrifugation, and was washed 3 times with distilled water followed by centrifugation each time to isolate the resin. The pH of the resulting 5% solids resin dispersion M2 was 6.0.

##### M3

To 14.6 g of solution A were added 25.4 g of distilled water and 20 g of Amberlite™ IR120<sup>+</sup> strongly acidic gel-type ion exchange resin. The mixture was stirred for five minutes, and the resin particles were separated from the liquid phase. The resin particles were washed with distilled, de-ionized water until the pH of a 20% resin slurry was 4.9. Five grams of the resulting developer loaded resin particles were added to 35 g of a solution containing 0.067 g of cetyltrimethylammonium bromide and 0.09 g of sodium sulfite. This slurry was sheared for 15 minutes with a rotor-stator mixer at ca. 15000 RPM. The resulting slurry was milled for 150 minutes with 120 cc of 1.8 mm zirconium oxide beads in an 8 oz jar to produce ion-exchanged developer M3.

##### M4

This ion exchange resin was prepared in the same manner as sample M1 except that DEV-2 was used in place of DEV-1 in solution A.

##### M5

This ion exchange resin was prepared in the same manner as sample M1 except that DEV-3 was used in place of DEV-1 in solution A.

##### M6

This ion exchange resin was prepared in the same manner as sample M1 except that DEV-4 was used in place of DEV-1 in solution A.

##### M7

Anionic blocked developer DEV-5 was exchanged to a quaternary ammonium resin as follows. Dowex<sup>R</sup> SBR (Cl<sup>-</sup> Form, Type1, Spherical Beads (strong base; styrene-DVB copolymer; trimethylbenzyl ammonium active group; total exchange capacity=3.1 meq/g) ion-exchange resin was milled to generate a dispersion with an average particle size of 0.7 um. To 38 ml of distilled water that had been purged with nitrogen was added 0.48 g of sodium sulfite, and 2 g of DEV-5. To 50 ml of distilled, nitrogen purged water was added 5 g of dried Dowex<sup>R</sup> SBR (Cl<sup>-</sup>) producing a smooth dispersion. The solution of DEV-5 was added to the resin dispersion, and stirred for 48 hours. The work-up of the developer resin was identical to M2.

##### P1

Direct synthesis of ion exchange resin particles with the desired particle size was also employed. Ion exchange resin particles were synthesized in the following manner. A copolymer resin comprising 85 wt % styrene, and 15 wt % divinylbenzene was synthesized by the suspension polymerization technique (McCaffery, Edward M.; *Laboratory Preparation for Macromolecular Chemistry*, McGraw-Hill, Inc., 1970.). The reaction conditions produced a narrow size distribution of particles with the mean size of 3 um. The beads were treated with sulfuric acid at elevated temperatures for 9 hours, thoroughly washed with distilled water, and dried. The level of sulfonation was 6 meq/g. To 30 ml of water was added 0.48 g of sodium sulfite followed by a 20 minute purge with nitrogen. To the purged solution was added 5 g of the 3 um sized sulfonated beads, and 8.5 g of DEV-1. The dispersion was stirred for 4 hours. The isolation procedure of P1 was identical to M2.

##### P2

The procedure for obtaining 1.5 um size resin beads is the same procedure as used in the resin preparation for the P1 example except that more stabilizer was used in this preparation, in order to obtain the smaller resin bead size. The sulfonation of the resin, and work-up procedure was identical to the one used in the P1 example. In this case the sulfonation level on the resin was 5.1 meq/g. The ion-

37

exchange procedure was identical to P1, keeping the molar ratio of sulfonic acid to DEV-1 constant in this preparation. P3

A sample of 1.5 micron resin particles were loaded with developer in the identical manner as for P2, except the molar ratio of sulfonic acid to DEV-1 was 1:0.125.



The following silver halide emulsion was prepared.

E1

A silver halide tabular emulsion with a composition of 97% silver bromide and 3% silver iodide was prepared by conventional means. The resulting emulsion had an equivalent circular diameter of 0.6 microns and a thickness of 0.09 microns. This emulsion was spectrally sensitized to green light and then chemically sensitized for optimum performance.

The following coupler dispersion was prepared.

C1

An oil based coupler dispersion was prepared by conventional methods containing coupler COUP-1 and tricresyl phosphate at a weight ratio of 1:0.5.

38

## EXAMPLE 2

## Processing of Color Paper with Materials of this Invention

This example demonstrates coatings containing developer loaded ion exchange particles embedded in a separate layer on a support are suitable for development of color print material. Ion-exchanged developer donor coatings were prepared containing, on a 1 m<sup>2</sup> basis: 0.65 g of DEV-1 from P3 and 4.31 g of de-ionized gelatin. Samples of Ektacolor Edge7 Color Paper were exposed to white light through a 0-4 neutral density step tablet and processed in the following manner. A thin layer (30 microns) of 0.5 M Na<sub>2</sub>CO<sub>3</sub> solution was uniformly applied to the color paper, and brought in contact with the ion-exchanged developer laminate. The coatings were passed through a set of pinch rollers, and heated for 10" at 50° C., then peeled apart, fixed, and washed. Status A reflection densities are shown in Table I. The inventive laminate processing material gave color paper images that were excellent in fog, latitude, and image discrimination.

TABLE I

| Results of processing color paper with a coating of the invention |                  |      |      |
|-------------------------------------------------------------------|------------------|------|------|
|                                                                   | Status A density | Dmin | Dmax |
| red density                                                       | 0.07             | 2.53 |      |
| green density                                                     | 0.09             | 2.49 |      |
| blue density                                                      | 0.14             | 2.43 |      |

## EXAMPLE 3

## Processing of Color Negative Film with Materials of this Invention

This example demonstrates coatings containing developer loaded ion exchange particles embedded in a binder are suitable for development of color negative film. Ion-exchanged developer donor coatings were prepared containing, on a 1 m<sup>2</sup> basis: 0.65 g of DEV-1 from P3 and 4.31 g of de-ionized gelatin. Samples of a 400 speed color negative film were exposed to white light through a 0-4 neutral density step tablet, and processed in the following manner. The exposed color negative film was immersed for 15 seconds in 1 M KOH and brought in contact with the ion-exchanged developer donor. The coatings were passed through a set of pinch rollers and held at room temperature for 60 seconds, then peeled apart, fixed and washed, to reveal a neutral negative image. Status M transmission densities are shown in Table II. The inventive laminate processing material gave color negative images that were excellent in fog, latitude, and image discrimination.

COUP-1



TABLE II

| Results of processing color negative film with a coating of the invention |      |      |
|---------------------------------------------------------------------------|------|------|
| Status M density                                                          | Dmin | Dmax |
| red density                                                               | 1.0  | 2.34 |
| green density                                                             | 1.35 | 2.84 |
| blue density                                                              | 1.70 | 2.94 |

## EXAMPLE 4

## Demonstration of Improved Image Formation

A comparative coating composition C-1 coated on a transparent film support contained 43.1 mg/dm<sup>2</sup> of de-ionized gelatin, 0.78 mg/dm<sup>2</sup> of hardener HAR-1, and 32.3 mg/dm<sup>2</sup> of DEV-1 from an aqueous solution of the free salt. An inventive coating composition I-1 coated on the same transparent film support contained 43.1 mg/dm<sup>2</sup> de-ionized gelatin, 0.78 mg/dm<sup>2</sup> of hardener HAR-1, and 28.8 mg/dm<sup>2</sup> of DEV-1 from composition P1. Coatings of Kodacolor Gold Plus 100 film were exposed with a 5500 K light source through a 0-4 neutral density step tablet and a Wratten<sup>TM</sup> 2B filter for  $\frac{1}{100}$  second. The exposed film was immersed for 10 seconds in a 5 weight percent KOH activator with 0.2 weight percent Triton X 100 surfactant and then laminated to the experimental processing materials through a set of pinch rollers. This composition was held for 60 seconds at 25° C., peeled apart, and then fixed and washed. The Status M transmission densities were measured and are summarized in Table III. It is clear from the table that the inventive laminate gave a superior image density range than the comparative coating in all three color records.

TABLE III

| Results of processing a color negative film with coatings containing DEV-1 |            |               |                 |                |
|----------------------------------------------------------------------------|------------|---------------|-----------------|----------------|
| coating                                                                    | type       | red Dmin/Dmax | green Dmin/Dmax | blue Dmin/Dmax |
| C-1                                                                        | comparison | 0.97/1.79     | 1.45/2.22       | 2.26/3.67      |
| I-1                                                                        | invention  | 1.12/2.68     | 1.46/2.46       | 2.30/4.05      |



HAR-1

## EXAMPLE 5

## Demonstration of Improved Raw Stock Incubation Stability

The coatings from Example 4 were placed into sealed bags and incubated in an oven for 1 week at 38° C. and 50% relative humidity. The DEV-1 in fresh and incubated coatings were enzymatically removed from the support, oxidized with potassium ferricyanide at pH 10, and reacted with coupler COUP-2 to produce a dye. The dye amount was then quantified in a 1 cm cell at circa 568 nm with a spectrophotometer and compared to known standards. In this way, the amount of DEV-1 in the coatings was determined. The data in Table IV show that the inventive coating had less loss of developer DEV-1 than the comparative coating. This is because the ion exchange resin stabilizes and protects the developer moiety from oxidation with the environment.

TABLE IV

| Results of raw stock incubation test |            |                                  |  |
|--------------------------------------|------------|----------------------------------|--|
| coating                              | type       | DEV-1 remaining after incubation |  |
| C-1                                  | comparison | 91.2%                            |  |
| I-1                                  | invention  | 99.8%                            |  |

COUP-2



## EXAMPLE 6

## Demonstration of Improved Physical Properties

The coatings from the Example 4 were immersed in a bath of distilled water for 2 minutes at 40° C. They were then removed from the bath and dried. Upon inspection and in comparison to the unprocessed coatings, the comparative coating was completely removed while the inventive coating was intact and unchanged. Measurements to verify the remaining DEV-1 levels were performed as in Example 5. The results are shown in Table V, and indicate the robustness of the materials of this invention. The free developer of the comparative coating interfered with the ability of the hardener to cross-link the gelatin binder in the coating. For this reason, the coating dissolved in the warm water and was removed. The ion exchange resin was able to stabilize the developer such that it did not interfere with the hardening reaction. Thus, the inventive coating remained intact. In addition, the ion exchange resin ballasted the developer into the coating, so that the free developer portion did not wander out of the coating and into the water bath. This is another advantage of the ion exchange materials of this invention.

TABLE V

| Stability of coatings in warm water |            |                                   |                        |
|-------------------------------------|------------|-----------------------------------|------------------------|
| coating                             | type       | disposition of coating after bath | active DEV-1 remaining |
| C-1                                 | comparison | removed                           | 0%                     |
| I-1                                 | invention  | intact                            | 98%                    |

## EXAMPLE 7

## Color photographic compositions with improved developer solubility

A set of coatings containing ion exchanged developers embedded in a photosensitive layer were prepared, exposed and processed as follows. Coatings were prepared containing on a 1 m<sup>2</sup> basis: 0.54 g of silver from silver halide emulsion E1, 0.32 g of magenta dye-forming coupler C1, 0.27 g of developer from the ion-exchanged developer source indicated in Table VI, and 4.04 g of de-ionized gelatin. The resulting coatings were exposed through a 0-4 neutral density step tablet and a Wratten 9<sup>TM</sup> filter for 1" with a 5500K light source.

The set of coatings were processed through a 5 minute pre-bath of distilled water, then immersed in a 0.5M sodium carbonate solution at 60° F. for 30 seconds, fixed, washed

and dried. Photographic performance is described in Table VI. Photographic speed was defined as the exposure at which the density above Dmin is 20% of the average gradient from that point to 0.6 log E greater exposure. A comparison coating of DEV-1 was also included which was prepared with the same format except the developer was added using Solution A. This coating did not contain ion-exchange particles. This distilled water pre-soaking experiment was used to demonstrate that the ion-exchange polymer adequately limits diffusion of the developer prior to immersion in the activator solution. Because the low pH of the pre-soak bath does not favor silver halide development, mobile developer species are washed out of the coatings without developing exposed silver halide emulsion grains. Subsequent immersion in the activator solution results in image formation from any remaining developer. The results in Table VI show that pre-soaking comparison coating using the Solution A source (which does not contain the ion-exchanged polymer) led to nearly complete loss of developer from the coating. As a result, only an extremely faint image was observed upon subsequent treatment with the activator solution. In contrast, the photographic performance of coatings containing ion-exchanged developer sources were not substantially affected by the pre-soak treatment. These results clearly demonstrate the usefulness of the ion-exchange polymers to limit unwanted diffusion of developer species incorporated in silver halide films.

TABLE VI

| Photographic results of pre-soaked coatings |            |      |      |                |
|---------------------------------------------|------------|------|------|----------------|
| DEV-1 source                                | type       | Dmin | Dmax | speed          |
| Solution A                                  | comparison | 0.03 | 0.21 | not measurable |
| M3                                          | invention  | 0.05 | 1.92 | 240            |
| M1                                          | invention  | 0.08 | 2.57 | 251            |
| M2                                          | invention  | 0.05 | 1.91 | 239            |
| P1                                          | invention  | 0.06 | 1.85 | 254            |

## EXAMPLE 8

Color Photographic Compositions with Improved Shelf Life

This example demonstrates improvements in photographic performance and shelf life are obtained when ion exchanged developer sources are embedded in a photosensitive layer. Samples of Amberlite IR120<sup>+</sup> ion exchange resin were loaded with developing agents DEV-2, DEV-3, and DEV-4 in the same manner as for M1. These are preparations M4 through M6. Coatings were prepared containing on a 1 m<sup>2</sup> basis: 0.54 g of silver from silver halide emulsion E1, 0.32 g of magenta dye-forming coupler C1, and 0.16 g of DEV-1 from P3. The resulting coatings were exposed through a 0-4 neutral density step tablet and a Wratten 9<sup>TM</sup> filter for 1" with a 5500K light source. Processing was immersion in a 0.5 M sodium carbonate solution at 60° F. for 30 seconds, fixed, washed and dried. Photographic performance is described in Table VII. Photographic speed was defined as the exposure at which the density above Dmin is 20% of the average gradient from that point to 0.6 log E greater exposure.

Comparison coatings were prepared except the developing agent was added from solution rather than including the ion-exchange resin. The coatings were exposed and processed as described above. A second set of coatings was incubated for four weeks at 120° F. and 50% RH prior to exposure and processing. Photographic performance is described in Table VII. The % discrimination was calculated

as the ratio of the difference between Dmax and Dmin of the incubated coating and the freshly processed coating. The results in Table VII demonstrate that the ion-exchanged developer resins provided similar or superior fresh image discrimination, and speed relative to comparison coatings which did not contain the ion-exchange resin. No image was observed with any of the incubated comparison coatings. Up to 95% of the initial image was retained when the ion exchange resin was employed to stabilize the color developer.

TABLE VII

| Example 8 photographic results |            |            |            |             |                                     |
|--------------------------------|------------|------------|------------|-------------|-------------------------------------|
| developer source               | type       | fresh Dmin | fresh Dmax | fresh speed | % discrimination for 4 week 120° F. |
| M1                             | invention  | 0.06       | 2.71       | 251         | 94                                  |
| Solution A                     | comparison | 0.05       | 2.41       | 214         | 0 (no image)                        |
| M4                             | invention  | 0.035      | 0.54       | 194         | 85                                  |
| DEV-2 solution                 | comparison | 0.045      | 0.48       | 193         | 0 (no image)                        |
| M5                             | invention  | 0.069      | 2.61       | 230         | 72                                  |
| DEV-3 solution                 | comparison | 0.056      | 2.28       | 230         | 0 (no image)                        |
| M6                             | invention  | 0.085      | 2.62       | 221         | 95                                  |
| DEV-4 solution                 | comparison | 0.067      | 2.60       | 143         | 0 (no image)                        |

## EXAMPLE 9

Ion Exchange Materials Processed with a Variety of Activator Solutions

This example demonstrates coatings containing ion exchanged developer sources embedded in a photosensitive layer may be processed with different activator solutions. Coatings were prepared containing on a 1 m<sup>2</sup> basis: 0.54 g of silver from silver halide emulsion E1, 0.32 g of magenta dye-forming coupler C1, and 0.16 g of DEV-1 from P3. The coatings were exposed as described in example 7 and were processed in the following activators at 60° F. for the time indicated in Table VIII. Photographic performance is described in Table VIII. These results demonstrate that a number of different activator solutions may be used to obtain similar photographic performance.

TABLE VIII

| Processing of materials with different activator solutions |               |       |       |       |
|------------------------------------------------------------|---------------|-------|-------|-------|
| activator composition                                      | time, seconds | Dmin  | Dmax  | speed |
| 0.5 M Na <sub>2</sub> CO <sub>3</sub>                      | 30            | 0.040 | 1.63  | 256   |
| 1 M NaOH                                                   | 30            | 0.073 | 1.87  | 248   |
| 0.1 M NaOH                                                 | 30            | 0.065 | 1.89  | 253   |
| 1 M NaCl at pH 12                                          | 30            | 0.057 | 0.73  | 250   |
| 1M NaCl at pH 12                                           | 60            | 0.058 | 1.29  | 251   |
| 0.0325 M Na <sub>2</sub> HPO <sub>4</sub> at pH 12         | 30            | 0.053 | 0.656 | 255   |
| 0.0325 M Na <sub>2</sub> HPO <sub>4</sub> at pH 12         | 60            | 0.060 | 1.227 | 266   |

## EXAMPLE 10

Color Photographic Composition Containing a Blocked Developer

This example demonstrates stabilization of a blocked developer using anionic-exchanged resin particles embedded in a photosensitive layer. Anionic blocked developer DEV-5 was exchanged to a quaternary ammonium resin as given in preparation M7. Coatings were prepared containing, on a 1 m<sup>2</sup> basis, 0.54 g of silver from silver

halide emulsion E2, 0.32 g of magenta dye-forming coupler C1, 0.55 g of DEV-5 from resin M7, 0.004 mmol of nitric acid, and 3.96 g of de-ionized gelatin. The coating was exposed as described in example 7. The coating was heated for 20 seconds at 160° C. to generate free developer and otherwise processed as described in example 7. A magenta-colored negative image was observed.

## EXAMPLE 11

## Activation of Layers with a Very Low Volume

This example demonstrates coatings containing developer loaded ion exchange particles embedded in a photosensitive layer are suitable for development when activated with a thin layer of liquid sufficient liquid to swell the emulsion layer. A sample of the coating containing M3 described in Example 7 was exposed and processed as described in Example 7 except the activator solution was uniformly applied in a thin layer (10 microns) sufficient to swell the light sensitive layer. Results shown in Table IX demonstrate that the ion-exchanged developers are a useful developer source for development schemes utilizing minimal activator solution usage.

TABLE IX

| Results of activation with a minimal amount of fluid |      |      |       |
|------------------------------------------------------|------|------|-------|
| DEV-1 source                                         | Dmin | Dmax | speed |
| M5                                                   | 0.11 | 2.08 | 248   |
| Solution A                                           | 0.22 | 2.35 | 220   |

## EXAMPLE 12

## Images Obtained From Layers Containing Ion Exchanged Materials

This example demonstrates developer loaded ion exchange particles embedded in a non-photosensitive layer of color negative film may be processed using an activator solution. A 100 speed color negative film element was prepared which contained a non-imaging overcoat with, on a 1 m<sup>2</sup> basis: 0.65 g of DEV-1 from P1 and 3.96 g of de-ionized gelatin. Samples of this film were loaded in a camera and image-wise exposed. The exposed film was processed as described in Example 7. The resulting film strip was scanned using a PhotoCD scanner, the images were viewed using Photoshop 4.0, and printed with a Kodak DS8650, a thermal printer. High quality color images were obtained.

The invention has been described in detail with particular reference to certain preferred embodiments thereof, but it will be understood that variations and modifications can be effected within the spirit and scope of the invention.

What is claimed is:

1. A sheet comprising a binder having dispersed therein particles of a photographically useful agent ionically bound to an ionic exchange matrix, wherein said sheet is not a photographic element comprising a silver halide emulsion layer.
2. A sheet according to claim 1, wherein the photographically useful reducing agent is a photographic developer, a blocked developer, a developer precursor, an electron transfer agent, a blocked electron transfer agent or an electron transfer agent precursor.
3. A sheet according to claim 1, wherein the ion exchange matrix is a natural or synthetic resin.
4. A sheet according to claim 3, wherein the ion exchange matrix is an organic synthetic resin.
5. A sheet according to claim 4, wherein the ion exchange matrix is a cationic ion exchange resin.

6. A sheet according to claim 5, wherein the cationic ion exchange resin carries one or more of the following ionic groups: SO<sub>3</sub><sup>-</sup>, COO<sup>-</sup>, PO<sub>3</sub><sup>2-</sup>, HPO<sub>2</sub><sup>-</sup>, AsO<sub>2</sub><sup>-</sup>, SeO<sub>3</sub><sup>-</sup>.

7. A sheet according to claim 6, wherein the cationic ion exchange resin carries SO<sub>3</sub><sup>-</sup> ionic groups.

8. A sheet according to claim 6, wherein the cationic ion exchange resin carries COO<sup>-</sup> ionic groups.

9. A sheet according to claim 6, wherein the cationic ion exchange resin is a sulfonated copolymer derived from styrene and divinylbenzene having a sulfonation level between about 3 to about 5 meq/g.

10. A sheet according to claim 4, wherein the ion exchange matrix is an anionic ion exchange resin.

11. A sheet according to claim 10, wherein the anionic ion exchange resin carries one or more of the following ionic groups:



12. A sheet according to claim 10, wherein the anionic ion exchange resin comprises a copolymer derived from styrene and divinylbenzene containing trimethylbenzylammonium chloride.

13. A sheet according to claim 1, wherein the photographically useful reducing agent is a developer.

14. A sheet according to claim 1, wherein the photographically useful reducing agent is a blocked developer.

15. A sheet according to claim 14, wherein the blocked developer releases a p-phenylenediamine.

16. A sheet according to claim 13, wherein the developer is a color developer.

17. A sheet according to claim 13, wherein the developer is a blocked color developer.

18. A sheet according to claim 16, wherein the color developer is a p-phenylenediamine or p-aminophenol.

19. A sheet according to claim 18, wherein the color developer is a p-phenylenediamine.

20. A sheet according to claim 1 further comprising a binder.

21. A sheet according to claim 20, wherein the binder comprises gelatin, poly(vinyl alcohol), or a cellulose derivative.

22. A sheet according to claim 1 or claim 20, which further comprises a support.

23. A sheet according to claim 22, wherein the support comprises a cellulose ester, poly(ethylene terephthalate) or poly(ethylene naphthalate).

24. A sheet according to claim 20, wherein the ionic exchange matrix comprises particles with average particle size less than 10  $\mu\text{m}$  in diameter.

25. A sheet according to claim 24, wherein the ionic exchange matrix comprises particles with average particle size less than 5  $\mu\text{m}$  in diameter.

26. A sheet according to claim 1, wherein the ion exchange matrix comprises a water-insoluble polymer.

27. A sheet according to claim 1, wherein the photographically useful compound is present in an amount of about 5 to about 100 mol percent of the ion exchange stoichiometric capacity.

28. A method of processing a photographic element comprising at least one silver halide light-sensitive emulsion layer which comprises contacting the element with (a) a processing solution and (b) a sheet comprising a photographically useful reducing agent ionically bound to ion exchange matrix.

**45**

**29.** A method of processing a photographic element comprising at least one silver halide light-sensitive emulsion layer which comprises contacting the element with (a) a processing solution having a pH of about 8-13 and (b) a sheet comprising a photographically useful reducing agent 5 ionically bound to an ionic exchange matrix.

**30.** A method of processing a photographic element comprising at least one silver halide light-sensitive emulsion layer which comprises contacting the element with (a) a processing solution having an ionic strength of greater than 10 0.001 M and (b) a sheet comprising a photographically useful reducing agent ionically bound to an ion exchange matrix.

**31.** A method of processing a photographic element comprising at least one silver halide light-sensitive layer 15 which comprises contacting the element with (a) a sheet comprising a photographically useful reducing agent ionically bound to an ion exchange matrix and (b) with thermal energy to elevate the temperature above 50° C.

**32.** A method of imaging comprising the steps of: 20 forming an image in an imagewise exposed light-sensitive silver halide element by the method of claim **28, 29, 30** or **31**;

**46**

scanning said formed image to form a first electronic image representation from said formed image;

digitizing said first electronic image to form a digital image;

modifying said digital image to form a second electronic image representation; and

transforming, storing, transmitting, printing or displaying said second electronic image representation.

**33.** A method of forming an image comprising the steps of:

forming an image in an imagewise exposed light-sensitive silver halide element by a method of claim **28, 29, 30** or **31**;

scanning said formed image to form an electronic image representation from said formed image; and

transforming, storing, transmitting, printing or displaying said electronic image representation.

\* \* \* \* \*